

# United States Patent [19]

Hoyen

[11] 4,395,478

[45] Jul. 26, 1983

- [54] **DIRECT-POSITIVE CORE-SHELL EMULSIONS AND PHOTOGRAPHIC ELEMENTS AND PROCESSES FOR THEIR USE**
- [75] Inventor: **Harry A. Hoyen**, Webster, N.Y.
- [73] Assignee: **Eastman Kodak Company**, Rochester, N.Y.
- [21] Appl. No.: **320,902**
- [22] Filed: **Nov. 12, 1981**
- [51] Int. Cl. 3 ..... **G03C 1/34**
- [52] U.S. Cl. ..... **430/217; 430/503; 430/409; 430/410; 430/375; 430/378; 430/377; 430/542; 430/547; 430/550; 430/598; 430/603; 430/605; 430/608; 430/940; 430/642**
- [58] Field of Search ..... **430/608, 940, 409, 596-598, 430/567, 642, 603, 605, 542, 547, 410, 375, 378, 503, 217, 377, 550**

[56]

## References Cited

### U.S. PATENT DOCUMENTS

- 3,713,832 1/1973 Shiba et al. ..... 430/940  
3,854,953 12/1974 Shiba et al. ..... 430/606

### FOREIGN PATENT DOCUMENTS

- 2323462 11/1973 Fed. Rep. of Germany ..... 430/596  
1423542 2/1976 United Kingdom ..... 430/596

Primary Examiner—Won H. Louie, Jr.

Attorney, Agent, or Firm—Carl O. Thomas

[57]

## ABSTRACT

A radiation-sensitive emulsion for use in forming a direct-positive image is disclosed. The emulsion is comprised of core-shell silver halide grains. The shell portions of the grains contain polyvalent metal ions to reduce rereversal.

**24 Claims, 1 Drawing Figure**

U.S. Patent

Jul. 26, 1983

4,395,478



*FIG. 1*

**DIRECT-POSITIVE CORE-SHELL EMULSIONS  
AND PHOTOGRAPHIC ELEMENTS AND  
PROCESSES FOR THEIR USE**

This invention relates to improved direct-positive core-shell emulsions and to photographic elements incorporating these emulsions. The invention further relates to processes of obtaining direct-positive images from imagewise exposed photographic elements.

**BACKGROUND OF THE INVENTION**

Photographic elements which produce images having an optical density directly related to the radiation received on exposure are said to be negative-working. A positive photographic image can be formed by producing a negative photographic image and then forming a second photographic image which is a negative of the first negative—that is, a positive image. A direct-positive image is understood in photography to be a positive image that is formed without first forming a negative image. Direct-positive photography is advantageous in providing a more straight-forward approach to obtaining positive photographic images.

A conventional approach to forming direct-positive images is to use photographic elements employing internal latent image-forming silver halide grains. After imagewise exposure, the silver halide grains are developed with a surface developer—that is, one which will leave the latent image sites within the silver halide grains substantially unrevealed. Simultaneously, either by uniform light exposure or by the use of a nucleating agent, the silver halide grains are subjected to development conditions that would cause fogging of a negative-working photographic element. The internal latent image-forming silver halide grains which received actinic radiation during imagewise exposure develop under these conditions at a slow rate as compared to the internal latent image-forming silver halide grains not imagewise exposed. The result is a direct-positive silver image. In color photography, the oxidized developer that is produced during silver development is used to produce a corresponding direct-positive dye image. Multi-color direct-positive photographic images have been extensively investigated in connection with image transfer photography.

Direct-positive internal latent image-forming emulsions can take the form of halide-conversion type emulsions. Such emulsions are illustrated by Knott et al U.S. Pat. No. 2,456,943 and Davey et al U.S. Pat. No. 2,592,250.

More recently the art has found it advantageous to employ core-shell emulsions as direct positive internal latent image-forming emulsions. An early teaching of core-shell emulsions is provided by Porter et al U.S. Pat. No. 3,206,313, wherein a coarse grain monodispersed chemically sensitized emulsion is blended with a finer grain emulsion. The blended finer grains are Ostwald ripened onto the chemically sensitized larger grains. A shell is thereby formed around the coarse grains. The chemical sensitization of the coarse grains is "buried" by the shell within the resulting core-shell grains. Upon imagewise exposure latent image sites are formed at internal sensitization sites and are therefore also internally located. The primary function of the shell structure is to prevent access of the surface developer to the internal latent image sites, thereby permitting low minimum densities.

The chemical sensitization of the core emulsion can take a variety of forms. One technique is to sensitize the core emulsion chemically at its surface with conventional sensitizers, such as sulfur and gold. Atwell et al 5 U.S. Pat. No. 4,035,185 teaches that controlling the ratio of middle chalcogen to noble metal sensitizers employed for core sensitization can control the contrast produced by the core-shell emulsion. Another technique that can be employed is to incorporate a metal 10 dopant, such as iridium, bismuth, or lead, in the core grains as they are formed.

The shell of the core-shell grains need not be formed by Ostwald ripening, as taught by Porter et al, but can be formed alternatively by direct precipitation onto the 15 sensitized core grains. Evans U.S. Pat. Nos. 3,761,276, 3,850,637, and 3,923,513 teach that further increases in photographic speed can be realized if, after the core-shell grains are formed, they are surface chemically sensitized. Surface chemical sensitization is, however, limited to maintain a balance of surface and internal sensitivity favoring the formation of internal latent 20 image sites.

Direct-positive emulsions exhibit art-recognized disadvantages as compared to negative-working emulsions. Although Evans, cited above, has been able to increase photographic speeds by properly balancing internal and surface sensitivities, direct-positive emulsions have not achieved photographic speeds equal to the faster surface latent image forming emulsions. Second, direct-positive core-shell emulsions are limited in 25 their permissible exposure latitude. When exposure is extended, rereversal occurs. That is, in areas receiving extended exposure a negative image is produced. This is a significant limitation to in-camera use of direct-positive 30 photographic elements, since candid photography does not always permit control of exposure conditions. For example, a very high contrast scene can lead to rereversal in some image areas.

A schematic illustration of rereversal is provided in 35 FIG. 1, which plots density versus exposure. A characteristic curve (stylized to exaggerate curve features for simplicity of discussion) is shown for a direct-positive emulsion. When the emulsion is coated as a layer on a support, exposed, and processed, a density is produced. The characteristic curve is the result of plotting various 40 levels of exposure versus the corresponding density produced on processing. At exposures below level A underexposure occurs and a maximum density is obtained which does not vary as a function of exposure. At exposure levels between A and B useful direct-positive 45 imaging can be achieved, since density varies inversely with exposure. If exposure occurs between the levels indicated by B and C, overexposure results. That is, density ceases to vary as a function of exposure in this range of exposures. If a subject to be photographed varies locally over a broad range of reflected light intensities, a photographic element containing the direct-positive emulsion can be simultaneously exposed in different areas at levels less than A and greater than B. The result may, however, still be aesthetically pleasing, 50 although highlight and shadow detail of the subject are both lost. If it is attempted to increase exposure for this subject, however, to pick up shadow detail, the result can be to increase highlight exposure to levels above C. When this occurs, rereversal is encountered. That is, the 55 areas overexposed beyond exposure level C appear as highly objectionable negative images, since density is now increasing directly with exposure. Useful exposure 60

latitude can be increased by more widely separating exposure levels A and B, but this is objectionable to the extent that it reduces contrast below optimum levels for most subjects. Therefore reduction in rereversal is most profitably directed to increasing the separation between exposure levels B and C so that overexposed areas are less likely to produce negative images. (In actual practice the various segments of the characteristic curve tend to merge more smoothly than illustrated.)

The use of inorganic salts of cadmium, manganese, and zinc as antifoggants is taught by Jones U.S. Pat. No. 2,839,405 and Sidebotham U.S. Pat. No. 3,488,709. Milton U.S. Pat. No. 3,761,266 teaches immersing a photographic element containing a core-shell emulsion having its shell comprised of silver chloride in a surface-image stabilizer bath containing cadmium chloride. Atwell U.S. Pat. No. 4,269,927 teaches that low levels of cadmium, lead, zinc, or copper dopants will increase the sensitivity of negative-working silver chloride emulsions.

#### SUMMARY OF THE INVENTION

In one aspect, this invention is directed to a radiation-sensitive emulsion particularly adapted to forming a direct-positive image comprised of a dispersing medium and silver halide grains capable of dispersing medium and silver halide grains capable of forming an internal latent image. The silver halide grains are comprised of a core and a shell. The shell incorporates in an amount sufficient to reduce rereversal one or more polyvalent metal ions chosen from the group consisting of manganese, copper, zinc, cadmium, lead, bismuth, and lanthanides.

In another aspect, this invention is directed to a photographic element comprised of a support and at least one radiation-sensitive emulsion layer comprised of a radiation-sensitive emulsion as described above.

In still another aspect, this invention is directed to processing in a surface developer an imagewise exposed photographic element as described above (1) in the presence of a nucleating agent or (2) with light-flashing of the exposed photographic element during processing.

It is an advantage of the present invention that wider exposure latitude can be realized without rereversal. In the examples below other advantages, such as reduced minimum density and increased speed, were also observed. In embodiments in which the shell portion of the grains contain chloride the present invention also permits the reduction of low intensity reciprocity failure and more rapid processing.

#### BRIEF DESCRIPTION OF THE DRAWINGS

The invention can be better understood by reference to the following detailed description of preferred embodiments considered in conjunction with the drawings, in which

FIG. 1 is a stylized characteristic curve of a direct-positive emulsion.

#### DESCRIPTION OF PREFERRED EMBODIMENTS

##### Sensitized Core-Shell Grains

It has been discovered that the amount of overexposure which can be tolerated without encountering rereversal in core-shell emulsions in forming direct-positive images can be increased by incorporating into the shells of core-shell grains polyvalent metal ion dopants. Divalent and trivalent cationic metal ion dopants

are specifically contemplated. Preferred divalent and trivalent cationic metal dopants for this purpose are manganese, copper, cadmium, zinc, lead, bismuth, and lanthanides. Lanthanides are elements 57 through 71 of the periodic table of elements. Erbium is a specifically preferred lanthanide. These metal ion dopants are generally effective at concentrations of from about  $10^{-3}$  to  $10^{-7}$  mole per mole of silver. Preferred concentration ranges are from  $5 \times 10^{-4}$  to  $5 \times 10^{-6}$  mole per mole of silver, with concentrations of from  $5 \times 10^{-5}$  to  $5 \times 10^{-6}$  mole per mole of silver being generally considered optimum. The metal ion dopants can be present singly or any combination in the shells in the concentration ranges indicated. The metals ions can be introduced into the shells by being present in the reaction vessel during precipitation or Ostwald ripening of the silver halide forming the shells onto the core grains. The metal ion dopants can be introduced into the reaction vessel as water soluble metal salts, such as divalent or trivalent metal halide salts. Techniques for incorporating metal ion dopants in similar concentrations in silver halide grains, but to achieve other modifying effects, are disclosed by Hochstetter U.S. Pat. No. 1,951,933, Mueller et al U.S. Pat. No. 2,950,972, McBride U.S. Pat. No. 3,287,136, Iwaosa et al U.S. Pat. No. 3,901,711, and Atwell U.S. Pat. No. 4,269,927.

Apart from the presence of polyvalent metal ion dopants incorporated into the shells of the core-shell grains, the core-shell emulsions of this invention can be identical to conventional core-shell emulsions, such as those described by Porter et al U.S. Pat. No. 3,206,313, Evans U.S. Pat. No. 3,761,276, 3,850,637, and 3,923,513, and Atwell U.S. Pat. No. 4,035,185, here incorporated by reference to provide a disclosure of such features. Accordingly, the following discussion is confined to certain core-shell emulsion, photographic element, and processing features which are particularly preferred and to those features which differ from the teachings of the Porter et al, Evans, and Atwell et al patents.

The formation of core-shell emulsions according to the present invention can begin with any convenient conventional sensitized core emulsion. The core emulsion can be comprised of silver bromide, silver chloride, silver chlorobromide, silver chloroiodide, silver bromo-iodide, or silver chlorobromoiodide grains. The grains can be coarse, medium, or fine and can be bounded by 100, 111, or 110 crystal planes. High aspect ratio tabular grain core-shell emulsions are the subject matter of Evans et al U.S. Ser. No. 320,891, filed currently here-with, entitled DIRECT REVERSAL EMULSIONS AND PHOTOGRAPHIC ELEMENTS USEFUL IN IMAGE TRANSFER FILM UNITS, commonly assigned and here incorporated by reference (now abandoned in favor of U.S. Ser. No. 431,912, filed Sept. 30, 1982). The present invention is applicable to the Evans et al emulsions. Prior to shelling, the core grains are preferably monodisperse. That is, the core grains prior to shelling preferably exhibit a coefficient of variation of less than 20% and for very high contrast applications optimally exhibit a coefficient of variation of less than 10%. The preferred completed core-shell emulsions of this invention exhibit similar coefficients of variations. (As employed herein the coefficient of variation is defined as 100 times the standard deviation of the grain diameter divided by the average grain diameter.) Although other sensitizations of the core emulsions are possible and contemplated, it is preferred to surface chemically sensitize the core emulsion grains with a

combination of middle chalcogen and noble metal sensitizers, as taught by Atwell et al, cited above. Additionally either middle chalcogen or noble metal sensitization can be employed alone. Sulfur, selenium, and gold are preferred sensitizers.

Although the sensitized core emulsion can be shelled by the Ostwald ripening technique of Porter et al, cited above, it is preferred that the silver halide forming the shell portion of the grains be precipitated directly onto the sensitized core grains by the double-jet addition technique. Double-jet precipitation is well known in the art, as illustrated by *Research Disclosure*, Vol. 176, December 1978, Item 17643, Section I, here incorporated by reference. *Research Disclosure* and its predecessor, Product Licensing Index, are publications of Industrial Opportunities Ltd., Homewell, Havant, Hampshire, PO9 1EF, United Kingdom. The halide content of the shell portion of the grains can take any of the forms described above with reference to the core emulsion. To improve developability it is preferred that the shell portion of the grains contain at least 80 mole percent chloride, the remaining halide being bromide or bromide and up to 10 mole percent iodide. (Except as otherwise indicated, all references to halide percentages are based on silver present in the corresponding emulsion, grain, or grain region being discussed.) Improvements in low intensity reciprocity failure are also realized when the shell portion of the core-shell grains is comprised of at least 80 mole percent chloride, as described above. For each of these advantages silver chloride is specifically preferred. On the other hand, the highest realized photographic speeds are generally recognized to occur with predominantly bromide grains, as taught by Evans, cited above. Thus, the specific choice of a preferred halide for the shell portion of the core-shell grains will depend upon the specific photographic application.

The silver halide forming the shell portion of the core shell grains must be sufficient to restrict developer access to the sensitized core portion of the grains. This will vary as a function of the ability of the developer to dissolve the shell portion of the grains during development. Although shell thickness as low as a few crystal lattice planes for developers having very low silver halide solvency are taught in the art, it is preferred that the shell portion of the core-shell grains be present in a molar ratio with the core portion of the grains of about 1:4 to 8:1, as taught by Porter et al and Atwell et al.

After precipitation of a shell portion onto the sensitized core grains to complete formation of the core-shell grains, the emulsions can be washed, if desired, to remove soluble salts. Conventional washing techniques can be employed, such as those disclosed by *Research Disclosure*, Item 17643, cited above, Section II, here incorporated by reference.

Since the core-shell emulsions are intended to form internal latent images, intentional sensitization of the surfaces of the core-shell grains is not essential. However, to achieve the highest attainable speeds, it is preferred that the core-shell grains be surface chemically sensitized, as taught by Evans and Atwell et al, cited above. Any type of surface chemical sensitization known to be useful with corresponding surface latent image-forming silver halide emulsions can be employed, such as disclosed by *Research Disclosure*, Item 17643, cited above, Section III. Middle chalcogen and/or noble metal sensitizations, as described by Atwell et al,

cited above, are preferred. Sulfur, selenium and gold are specifically preferred surface sensitizers.

The degree of surface chemical sensitization is limited to that which will increase the speed of the internal latent image-forming emulsion, but which will not compete with the internal sensitization sites to the extent of causing the location of latent image centers formed on exposure to shift from the interior to the surface of the tabular grains. Thus, a balance between internal and surface sensitization is preferably maintained for maximum speed, but with the internal sensitization predominating. Tolerable levels of surface chemical sensitization can be readily determined by the following test: A sample of the high aspect ratio tabular grain internal latent image-forming silver halide emulsion of the present invention is coated on a transparent film support at a silver coverage of 4 grams per square meter. The coated sample is then exposed to a 500 watt tungsten lamp for times ranging from 0.01 to 1 second at a distance of 0.6 meter. The exposed coated sample is then developed for 5 minutes at 20° C. in Developer Y below (an "internal type" developer, note the incorporation of iodide to provide access to the interior of the grain), fixed, washed, and dried. The procedure described above is repeated with a second sample identically coated and exposed. Processing is also identical, except that Developer X below (a "surface type" developer) is substituted for Developer Y. To satisfy the requirements of the present invention as being a useful internal latent image-forming emulsion the sample developed in the internal type developer, Developer Y, must exhibit a maximum density at least 5 times greater than the sample developed in the surface type developer, Developer X. This difference in density is a positive indication that the latent image centers of the silver halide grains are forming predominantly in the interior of the grains and are for the most part inaccessible to the surface type developer.

|                                | Grams |
|--------------------------------|-------|
| <u>Developer X</u>             |       |
| N—methyl-p-aminophenol sulfate | 2.5   |
| Ascorbic acid                  | 10.0  |
| Potassium metaborate           | 35.0  |
| Potassium bromide              | 1.0   |
| Water to 1 liter.              |       |
| <u>Developer Y</u>             |       |
| N—methyl-p-aminophenol sulfate | 2.0   |
| Sodium sulfite, desiccated     | 90.0  |
| Hydroquinone                   | 8.0   |
| Sodium carbonate, monohydrate  | 52.5  |
| Potassium bromide              | 5.0   |
| Potassium iodide               | 0.5   |
| Water to 1 liter.              |       |

The core-shell emulsions of the present invention can, if desired, be spectrally sensitized. For multicolor photographic applications red, green, or, optionally, blue spectral sensitizing dyes can be employed, depending upon the portion of the visible spectrum the core-shell grains are intended to record. For black-and-white imaging applications spectral sensitizing is not required, although orthochromatic or panchromatic sensitization is usually preferred. Generally, any spectral sensitizing or dye combination known to be useful with a negative-working silver halide emulsion can be employed with the core-shell emulsions of the present invention. Illustrative spectral sensitizing dyes are those disclosed in *Research Disclosure*, Item 17643, cited above, Section

IV. Particularly preferred spectral sensitizing dyes are those disclosed in *Research Disclosure*, Vol. 151, November 1976, Item 15162, here incorporated by reference. Although the emulsions can be spectrally sensitized with dyes from a variety of classes, preferred spectral sensitizing dyes are polymethine dyes, which include cyanine, merocyanine, complex cyanine and merocyanine (i.e., tri-, tetra-, and poly-nuclear cyanine and merocyanine), oxonol, hemioxonol, styryl, merostyryl, and streptocyanine dyes. Cyanine and merocyanine dyes are specifically preferred. Spectral sensitizing dyes which sensitize surface-fogged direct-positive emulsions generally desensitize both negative-working emulsions and the core-shell emulsions of this invention and therefore are not normally contemplated for use in the practice of this invention. Spectral sensitization can be undertaken at any stage of emulsion preparation heretofore known to be useful. Most commonly spectral sensitization is undertaken in the art subsequent to the completion of chemical sensitization. However, it is specifically recognized that spectral sensitization can be undertaken alternatively concurrently with chemical sensitization or can entirely precede chemical sensitization. Sensitization can be enhanced by pAg adjustment, including cycling, during chemical and/or spectral sensitization.

## Nucleating Agents

It has been found advantageous to employ nucleating agents in preference to uniform light exposure in processing. The term "nucleating agent" is employed herein in its art-recognized usage to mean a fogging agent capable of permitting the selective development of internal latent image-forming silver halide grains which have not been imagewise exposed, in preference to the development of silver halide grains having an internal latent image formed by imagewise exposure.

The core-shell emulsions of this invention preferably incorporate a nucleating agent to promote the formation of a direct-positive image upon processing. The nucleating agent can be incorporated in the emulsion during processing, but is preferably incorporated in manufacture of the photographic element, usually prior to coating. This reduces the quantities of nucleating agent required. The quantities of nucleating agent required can also be reduced by restricting the mobility of the nucleating agent in the photographic element. Large organic substituents capable of performing at least to some extent a ballasting function are commonly employed. Nucleating agents which include one or more groups to promote adsorption to the surface of the silver halide grains have been found to be effective in extremely low concentrations.

A preferred general class of nucleating agents for use in the practice of this invention are aromatic hydrazides. Particularly preferred aromatic hydrazides are those in which the aromatic nucleus is substituted with one or more groups to restrict mobility and, preferably, promote adsorption of the hydrazide to silver halide grain surfaces. More specifically, preferred hydrazides are those embraced by formula (I) below:



wherein

D is an acyl group:

$\phi$  is a phenylene or substituted (e.g., halo-, alkyl-, or alkoxy-substituted) phenylene group; and  
 M is a moiety capable of restricting mobility, such as an adsorption promoting moiety.

A particularly preferred class of phenylhydrazides are acylhydrazinophenylthioureas represented by formula (II) below.



wherein

15. *wherein*  
 15. R is hydrogen or an alkyl, cycloalkyl, haloalkyl, alkoxy-alkyl, or phenylalkyl substituent or a phenyl nucleus having a Hammett sigma-value-derived electron-withdrawing characteristic more positive than -0.30;

20  $R^1$  is a phenylene or alkyl, halo-, or alkoxy-substituted phenylene group;

$R^2$  is hydrogen, benzyl, alkoxybenzyl, halobenzyl, or alkylbenzyl;

25 R<sup>3</sup> is a alkyl, haloalkyl, alkoxyalkyl, or phenylalkyl substituent having from 1 to 18 carbon atoms, a cycloalkyl substituent, a phenyl nucleus having a Hammett sigma value-derived electron-withdrawing characteristic less positive than +0.50, or naphthyl.

30  $R^4$  is hydrogen or independently selected from among the same substituents as  $R^3$ ; or

$R^3$  and  $R^4$  together form a heterocyclic nucleus forming a 5- or 6-membered ring, wherein the ring atoms are chosen from the class consisting of nitrogen, carbon, oxygen, sulfur, and selenium atoms;

33 with the proviso that at least one of  $R^2$  and  $R^4$  must be hydrogen and the alkyl moieties, except as otherwise noted, in each instance include from 1 to 6 carbon atoms and the cycloalkyl moieties have from 3 to 10 carbon atoms.

As indicated by R in formula (II), preferred acylhydrazinophenylthioureas employed in the practice of this invention contain an acyl group which is the residue of a carboxylic acid, such as one of the acyclic carboxylic acids, including formic acid, acetic acid, propionic acid, butyric acid, higher homologues of these acids having up to about 7 carbon atoms, and halogen, alkoxy, phenyl and equivalent substituted derivatives thereof. In a preferred form, the acyl group is formed by an unsubstituted acyclic aliphatic carboxylic acid having from 1 to 5 carbon atoms. Specifically preferred acyl groups are formyl and acetyl. As between compounds which differ solely in terms of having a formyl or an acetyl group, the compound containing the formyl group exhibits higher nucleating agent activity. The alkyl moieties in the substituents to the carboxylic acids are contemplated to have from 1 to 6 carbon atoms, preferably from 1 to 4 carbon atoms.

In addition to the acyclic aliphatic carboxylic acids, it is recognized that the carboxylic acid can be chosen so that R is a cyclic aliphatic group having from about 3 to 10 carbon atoms, such as, cyclopropyl, cyclobutyl, cyclopentyl, cyclohexyl, methylcyclohexyl, cyclooctyl, cyclodecyl, and bridged ring variations, such as, bornyl and isobornyl groups. Cyclohexyl is a specifically preferred cycloalkyl substituent. The use of alkoxy, cyano, halogen, and equivalent substituted cycloalkyl substituents is contemplated.

As indicated by R<sup>1</sup> in formula (II), preferred acylhydrazinophenylthioureas employed in the practice of this invention contain a phenylene or substituted phenylene group. Specifically preferred phenylene groups are m- and p-phenylene groups. Exemplary of preferred phenylene substituents are alkoxy substituents having from 1 to 6 carbon atoms, alkyl substituents having from 1 to 6 carbon atoms, fluoro-, chloro-, bromo-, and iodo-substituents. Unsubstituted p-phenylene groups are specifically preferred. Specifically preferred alkyl moieties are those which have from 1 to 4 carbon atoms. While phenylene and substituted phenylene groups are preferred linking groups, other functionally equivalent divalent aryl groups, such as naphthalene groups, can be employed.

In one form  $R^2$  represents an unsubstituted benzyl group or substituted equivalents thereof, such as alkyl, halo-, or alkoxy-substituted benzyl groups. In the preferred form no more than 6 and, most preferably, no more than 4 carbon atoms are contributed by substituents to the benzyl group. Substituents to the benzyl group are preferably para-substituents. Specifically preferred benzyl substituents are formed by unsubstituted, 4-halo-substituted, 4-methoxy-substituted, and 4-methyl-substituted benzyl groups. In another specifically preferred form  $R^2$  represents hydrogen.

Referring again to formula (II), it is apparent that  $R^3$  and  $R^4$  can independently take a variety of forms. One specifically contemplated form can be an alkyl group or a substituted alkyl group, such as a haloalkyl group, alkoxyalkyl group, phenylalkyl group, or equivalent group, having a total of up to 18, preferably up to 12, carbon atoms. Specifically  $R^3$  and/or  $R^4$  can take the form of a methyl, ethyl, propyl, butyl, pentyl, hexyl, heptyl, octyl, nonyl, decyl or higher homologue group having up to 18 total carbon atoms; a fluoro-, chloro-, bromo-, or iodo-substituted derivative thereof; a methoxy, ethoxy, propoxy, butoxy or higher homologue alkoxy-substituted derivative thereof, wherein the total number of carbon atoms are necessarily at least 2 up to 18; and a phenyl-substituted derivative thereof, wherein the total number of carbon atoms is necessarily at least 7, as in the case of benzyl, up to about 18. In a specific preferred form  $R^3$  and/or  $R^4$  can take the form of an alkyl or phenylalkyl substituent, wherein the alkyl moieties are in each instance from 1 to 6 carbon atoms.

In addition to the acyclic aliphatic and aromatic forms discussed above, it is also contemplated that  $R^3$  and/or  $R^4$  can take the form of a cyclic aliphatic substituent, such as a cycloalkyl substituent having from 3 to 10 carbon atoms. The use of cyclopropyl, cyclobutyl, cyclopentyl, cyclohexyl, methylcyclohexyl, cyclooctyl, cyclodecyl and bridged ring variations, such as, bornyl and isobornyl groups, is contemplated. Cyclohexyl is a preferred cycloalkyl substituent. The use of alkoxy, cyano, halogen and equivalent substituted cycloalkyl substituents is contemplated.

$R^3$  and/or  $R^4$  can also be an aromatic substituent, such as, phenyl or naphthyl (i.e., 1-naphthyl or 2-naphthyl) or an equivalent aromatic group, e.g., 1-, 2-, or 6-9-anthryl, etc. As indicated in formula (II)  $R^3$  and/or  $R^4$  can take the form of a phenyl nucleus which is either electron-donating or electron-withdrawing, however phenyl nuclei which are highly electron-withdrawing may produce inferior nucleating agents. 65

The electron-withdrawing or electron-donating characteristic of a specific phenyl nucleus can be assessed by reference to Hammett sigma values. The phenyl nucleus

10

can be assigned a Hammett sigma value-derived electron-withdrawing characteristic which is the algebraic sum of the Hammett sigma value of its substituents (i.e., those of the substituents, if any, to the phenyl group).

- 5 For example, the Hammett sigma values of any substituents to the phenyl ring of the phenyl nucleus can be determined algebraically simply by determining from the literature the known Hammett sigma values for each substituent and obtaining the algebraic sum thereof.

10 Electron-withdrawing substituents are assigned positive sigma values, while electron-donating substituents are assigned negative sigma values.

15 Exemplary meta- and para-sigma values and procedures for their determination are set forth by J. Hine in *Physical Organic Chemistry*, second edition, page 87, published in 1962, H. VanBekkum, P. E. Verkade and B. M. Wepster in *Rec. Trav. Chim.*, Volume 78, page 815, published in 1959, P. R. Wells in *Chem. Revs.*, Volume 63, page 171, published in 1963, by H. H. Jaffé in *Chem. Revs.*, Volume 53, page 191, published in 1953, by M. J. S. Dewar and P. J. Grisdale in *J. Amer. Chem. Soc.*, Volume 84, page 3548, published in 1962, and by Barlin and Perrin in *Quart. Revs.*, Volume 20, page 75 et seq, published in 1966. For the purposes of this invention, ortho-substituents to the phenyl ring can be assigned to the published para-sigma values.

It is preferred that  $R^2$  and/or  $R^3$  be a phenyl nucleus having a Hammett sigma value-derived electron-withdrawing characteristic less positive than +0.50. It is specifically contemplated that  $R^2$  and/or  $R^3$  be chosen from among phenyl nuclei having cyano, fluoro-, chloro-, bromo-, iodo-, alkyl groups having from 1 to 6 carbon atoms, and alkoxy groups having from 1 to 6 carbon atoms, as phenyl ring substituents. Phenyl ring substituents are preferred in the para- or 4-ring position.

Rather than being independently chosen  $R^3$  and  $R^3'$  can together form, along with the 3-position nitrogen atom of the thiourea, a heterocyclic nucleus forming a 5- or 6-membered ring. The ring atoms can be chosen from among nitrogen, carbon, oxygen, sulfur and selenium atoms. The ring necessarily contains at least one nitrogen atom. Exemplary rings include morpholinyl, piperidino, pyrrolidinyl, pyrrolinyl, thiomorpholino, thiazolidinyl, 4-thiazolinyl, selenazolidinyl, 4-selenazolinyl, imidazolidinyl, imidazolinyl, oxazolidinyl and 4-oxazolinyl rings. Specifically preferred rings are saturated or otherwise constructed to avoid electron withdrawal from the 3-position nitrogen atom.

Acylhydrazinophenylthiourea nucleating agents and their synthesis are more specifically disclosed in Leone U.S. Pat. Nos. 4,030,925 and 4,276,364, here incorporated by reference. Variants of the acylhydrazinophenylthiourea nucleating agents described above are disclosed in von Konig U.S. Pat. No. 4,139,387 and Adachi et al. U.K. Patent Application No. 2,012,443A.

Another preferred class of phenylhydrazide nucleating agents are N-(acylhydrazinophenyl)thioamide nucleating agents, such as those indicated by formula (III) below:



65. wherein

R and R' are as defined in formula (II);  
 A is  $\equiv N-R^2$ ,  $-S-$  or  $-O-$ :

$Q^1$  represents the atoms necessary to complete a five-membered heterocyclic nucleus;  $R^2$  is independently chosen from hydrogen, phenyl, alkyl, alkylphenyl, and phenylalkyl; and the alkyl moieties in each instance include from 1 to 6 carbon atoms.

These compounds embrace those having a five-membered heterocyclic thioamide nucleus, such as a 4-thiazoline-2-thione, thiazolidine-2-thione, 4-oxazoline-2-thione, oxazolidine-2-thione, 2-pyrazoline-5-thione, pyrazolidine-5-thione, indoline-2-thione, 4-imidazoline-2-thione, etc. A specifically preferred subclass of heterocyclic thioamide nuclei is formed when  $Q^1$  is as indicated in formula (IV)



wherein

$X$  is  $=S$  or  $=O$ .

Specifically preferred illustrations of such values of  $Q^1$  are 2-thiohydantoin, rhodanine, isorhodanine, and 2-thio-2,4-oxazolidinedione nuclei. It is believed that some six-membered nuclei, such as thiobarbituric acid, may be equivalent to five-membered nuclei embraced within formula (III).

Another specifically preferred subclass of heterocyclic thioamide nuclei is formed when  $Q^1$  is as indicated in formula (V)



wherein

$L$  is a methine group;

$Z$  is  $=C(CH=CH_2)_n-N-R^3$  or  $=CH-C_6H_4-N-R^3$ ;

$R^3$  is an alkyl substituent;  $R^4$  is hydrogen; an alkyl,  $-N(R^5-R^6)$ , or an

alkoxy substituent;

$Z$  represents the nonmetallic atoms necessary to complete a basic heterocyclic nucleus of the type found in cyanine dyes;

$n$  and  $d$  are independently chosen from the integers 1 and 2;

$R^5$  and  $R^6$  are independently chosen from hydrogen, phenyl, alkyl, alkylphenyl, and phenylalkyl; and the alkyl moieties in each instance include from 1 to 6 carbon atoms.

The formula (V) values for  $Q^1$  provide a heterocyclic thioamide nucleus corresponding to a methine substituted form of the nuclei present above in formula (IV) values for  $Q^1$ . In a specifically preferred form the heterocyclic thioamide nucleus is preferably a methine substituted 2-thiohydantoin, rhodanine, isorhodanine, or 2-thio-2,4-oxazolidinedione nucleus. The heterocyclic thioamide nucleus of formula (V) is directly, or through an intermediate methine linkage, substituted with a basic heterocyclic nucleus of the type employed in

cyanine dyes or a substituted benzylidene nucleus.  $Z$  preferably represents the nonmetallic atoms necessary to complete a basic 5- or 6-membered heterocyclic nucleus of the type found in cyanine dyes having ring-forming atoms chosen from the class consisting of carbon, nitrogen, oxygen, sulfur, and selenium.

$N$ -(acylhydrazinophenyl)thioamide nucleating agents and their synthesis are more specifically disclosed in Leone et al U.S. Pat. No. 4,080,207.

Still another preferred class of phenylhydrazide nucleating agents are triazole-substituted phenylhydrazide nucleating agents. More specifically, preferred triazole-substituted phenylhydrazide nucleating agents are those represented by formula VI below:



wherein

$R$  and  $R'$  are as defined in formula (II);

$A^1$  is alkylene or oxalkylene;



$A^3$  is a triazolyl or benzotriazolyl nucleus;

the alkyl and alkylene moieties in each instance including from 1 to 6 carbon atoms.

Still more specifically preferred triazole-substituted phenylhydrazide nucleating agents are those represented by formula (VII) below:



wherein

$R$  is hydrogen or methyl;



$n$  is an integer of 1 to 4; and

$E$  is alkyl of from 1 to 4 carbon atoms.

Triazole-substituted phenylhydrazide nucleating agents and their synthesis are disclosed by Sidhu et al U.S. Pat. No. 4,278,748, here incorporated by reference. Comparable nucleating agents having a somewhat broader range of adsorption promoting groups are disclosed in corresponding U.K. Patent Application Ser. No. 2,011,391A.

The aromatic hydrazides represented by formulas (II), (III), and (VI) each contain adsorption promoting substituents. In many instances it is preferred to employ in combination with these aromatic hydrazides additional hydrazides or hydrazones which do not contain substituents specifically intended to promote adsorption to silver halide grain surfaces. Such hydrazides or hydra-

zones, however, often contain substituents to reduce their mobility when incorporated in photographic elements. These hydrazide or hydrazone can be employed as the sole nucleating agent, if desired.

Such hydrazides and hydrazone include those represented by formula (VIII) and (IX) below:



wherein T is an aryl radical, including a substituted aryl radical, T<sup>1</sup> is an acyl radical, and T<sup>2</sup> is an alkylidene radical and including substituted alkylidene radicals. Typical aryl radicals for the substituent T have the formula M-T<sup>3</sup>, wherein T<sup>3</sup> is an aryl radical (such as, phenyl, 1-naphthyl, 2-naphthyl, etc.) and M can be such substituents as hydrogen, hydroxy, amino, alkyl, alkylamino, arylamino, heterocyclic amino (amino containing a heterocyclic moiety), alkoxy, aryloxy, acyloxy, arylcarbonamido, alkylcarbonamido, heterocyclic carbonamido (carbonamido containing a heterocyclic moiety), arylsulfonamido, alkylsulfonamido, and heterocyclic sulfonamido (sulfonamido containing a heterocyclic moiety). Typical acyl radicals for the substituent T<sup>1</sup> have the formula



wherein Y can be such substituents as alkyl, aryl, and heterocyclic radicals, G can represent a hydrogen atom or the same substituent as Y as well as radicals having the formula



to form oxanyl radicals wherein A is an alkyl, aryl, or a heterocyclic radical. Typical alkylidene radicals for the substituent T<sup>2</sup> have the formula =CH-D wherein D can be a hydrogen atom or such radicals as alkyl, aryl, and heterocyclic radicals. Typical aryl substituents for the above-described hydrazides and hydrazone include phenyl, naphthyl, diphenyl, and the like. Typical heterocyclic substituents for the above-described hydrazides and hydrazone include azoles, azines, furan, thiophene, quinoline, pyrazole, and the like. Typical alkyl (or alkylidene) substituents for the above-described hydrazides and hydrazone have 1 to 22 carbon atoms including methyl, ethyl, isopropyl, n-propyl, isobutyl, n-butyl, t-butyl, amyl, n-octyl, n-decyl, n-dodecyl, n-octadecyl, n-eicosyl, and n-docosyl.

The hydrazides and hydrazone represented by formulas (VIII) and (IX) as well as their synthesis are disclosed by Whitmore U.S. Pat. No. 3,227,552, here incorporated by reference.

A secondary preferred general class of nucleating agents for use in the practice of this invention are N-substituted cycloammonium quaternary salts. A particularly preferred species of such nucleating agents is represented by formula (X) below:



wherein

10 Z<sup>1</sup> represents the atoms necessary to complete a heterocyclic nucleus containing a heterocyclic ring of 5 to 6 atoms including the quaternary nitrogen atoms, with the additional atoms of said heterocyclic ring being selected from carbon, nitrogen, oxygen, sulfur, and selenium;

j represents a positive integer of from 1 to 2;

a represents a positive integer of from 2 to 6;

20 X<sup>-</sup> represents an acid anion;

E<sup>2</sup> represents a member selected from (a) a formyl radical, (b) a radical having the formula



wherein each of L<sup>1</sup> and L<sup>2</sup>, when taken alone, represents a member selected from an alkoxy radical and an alkylthio radical, and L<sup>1</sup> and L<sup>2</sup>, when taken together, represent the atoms necessary to complete a cyclic radical selected from cyclic oxyacetals and cyclic thioacetals having from 5 to 6 atoms in the heterocyclic acetal ring, and (c) a 1-hydrazonoalkyl radical; and

E<sup>1</sup> represents either a hydrogen atom, an alkyl radical, an aralkyl radical, an alkylthio radical, or an aryl radical such as phenyl and naphthyl, and including substituted aryl radicals.

The N-substituted cycloammonium quaternary salt nucleating agents of formula (X) and their synthesis are disclosed by Lincoln and Heseltine U.S. Pat. Nos. 3,615,615 and 3,759,901. In a variant form E<sup>1</sup> can be a divalent alkylene group of from 2 to 4 carbon atoms joining two substituted heterocyclic nuclei as shown in formula (X). Such nucleating agents and their synthesis are disclosed by Kurtz and Harbison U.S. Pat. No. 3,734,738.

The substituent to the quaternized nitrogen atom of the heterocyclic ring can, in another variant form, itself form a fused ring with the heterocyclic ring. Such nucleating agents are illustrated by dihydroaromatic quaternary salts comprising a 1,2-dihydroaromatic heterocyclic nucleus including a quaternary nitrogen atom. Particularly advantageous 1,2-dihydroaromatic nuclei include such nuclei as a 1,2-dihydropyridinium nucleus. Especially preferred dihydroaromatic quaternary salt nucleating agents include those represented by formula (XI) below:



(XII)

wherein

Z represents the nonmetallic atoms necessary to complete a heterocyclic nucleus containing a heterocyclic ring of from 5 to 6 atoms including the quaternary nitrogen atom, with the additional atoms of said heterocyclic ring being selected from either carbon, nitrogen, oxygen, sulfur, or selenium;

n represents a positive integer having a value of from 1 to 2;

when n is 1, R represents a member selected from the group consisting of a hydrogen atom, an alkyl radical, an alkoxy radical, an aryl radical, an aryloxy radical, and a carbamido radical and,

when n is 2, R represents an alkylene radical having from 1 to 4 carbon atoms;

each of R<sup>1</sup> and R<sup>2</sup> represents a member selected from the group consisting of a hydrogen atom, an alkyl radical, and an aryl radical; and

X- represents an anion.

Dihydroaromatic quaternary salt nucleating agents and their synthesis are disclosed by Kurtz and Heseltine U.S. Pat. No. 3,719,494, here incorporated by reference.

A specifically preferred class of N-substituted cycloammonium quaternary salt nucleating agents are those which include one or more alkynyl substituents. Such nucleating agents include compounds within the generic structural definition set forth in formula (XII) below:



(XII)

wherein Z represents an atomic group necessary for forming a 5- or 6-membered heterocyclic nucleus, R<sup>1</sup> represents an aliphatic group, R<sup>2</sup> represents a hydrogen atom or an aliphatic group, R<sup>3</sup> and R<sup>4</sup>, which may be the same or different, each represents a hydrogen atom, a halogen atom, an aliphatic group, an alkoxy group, a hydroxy group, or an aromatic group, at least one of R<sup>1</sup>, R<sup>2</sup>, R<sup>3</sup> and R<sup>4</sup> being a propargyl group, a butynyl group, or a substituent containing a propargyl or butynyl group, X- represents an anion, n is 1 or 2, with n being 1 when the compound forms an inner salt.

Such alkynyl-substituted cycloammonium quaternary salt nucleating agents and their synthesis are illustrated by Adachi et al U.S. Pat. No. 4,115,122, here incorporated by reference.

The specific choice of nucleating agents can be influenced by a variety of factors. The nucleating agents of Leone cited above are particularly preferred for many applications, since they are effective at very low concentrations. Minimum concentrations as low as 0.1 mg of nucleating agent per mole of silver, preferably at least

0.5 mg per silver mole, and optimally at least 1 mg per silver mole are disclosed by Leone. The nucleating agents of Leone are particularly advantageous in reducing speed loss and in some instances permitting speed gain with increasing processing temperatures. When the nucleating agents of Leone are employed in combination with those of Whitmore speed variations as a function of temperature of processing can be minimized.

The aromatic hydrazide nucleating agents are generally preferred for use in photographic elements intended to be processed at comparatively high levels of pH, typically above 13. The alkynyl-substituted cycloammonium quaternary salt nucleating agents are particularly useful for processing at a pH of 13 or less. Adachi et al teaches these nucleating agents to be useful in processing within the pH range of from 10 to 13, preferably 11 to 12.5.

In addition to the nucleating agents described above additional nucleating agents have been identified which are useful in processing at pH levels in the range of from about 10 to 13. An N-substituted cycloammonium quaternary salt nucleating agent which can, one or more, contain alkynyl substituents is illustrative of one class of nucleating agents useful in processing below pH 13. Such nucleating agents are illustrated by formula (XIII) below:



(XIII)

wherein

Z<sup>1</sup> represents the atoms completing an aromatic carbocyclic nucleus of from 6 to 10 carbon atoms;

Y<sup>1</sup> and Y<sup>2</sup> are independently selected from among a divalent oxygen atom, a divalent sulfur atom, and

40



45 Z<sup>2</sup> represents the atoms completing a heterocyclic nucleus of the type found in cyanine dyes;

A is an adsorption promoting moiety;

m and n are 1 or 2; and

R<sup>1</sup>, R<sup>2</sup>, and R<sup>3</sup> are independently chosen from the group consisting of hydrogen, alkyl, aryl, alkaryl, and aralkyl and R<sup>1</sup> and R<sup>3</sup> are additionally independently chosen from the group consisting of acyl, alkenyl, and alkynyl, the aliphatic moieties containing up to 5 carbon atoms and the aromatic moieties containing 6 to 10 carbon atoms. A preferred processing pH when these nucleating agents are employed is in the range of from 10.2 to 12.0.

Nucleating agents of the type represented by formula (XIII) and their synthesis are disclosed by Baralle et al U.S. Ser. No. 207,530, filed Nov. 17, 1980, commonly assigned and here incorporated by reference (now U.S. Pat. No. 4,306,016).

Another class of nucleating agents effective in the pH range of from 10 to 13, preferably 10.2 to 12, are dihydrospiropyran bis-condensation products of salicylic aldehyde and at least one heterocyclic ammonium salt. In a preferred form such nucleating agents are represented by formula (XIV) below:

55



(XIV)

wherein  
 X and Y each independently represent a sulfur atom, a selenium atom or a  $-\text{C}(\text{R}^1\text{R}^2)-$  radical,  
 R<sup>1</sup> and R<sup>2</sup> independently represent lower alkyl of from 1 to 5 carbon atoms or together represent an alkylene radical of 4 to 5 carbon atoms,  
 R<sup>3</sup>, R<sup>4</sup>, R<sup>5</sup>, and R<sup>6</sup> each represent hydrogen, a hydroxy radical or a lower alkyl or alkoxy radical of from 1 to 5 carbon atoms,

Z<sup>1</sup> and Z<sup>2</sup> each represents the nonmetallic atoms completing a nitrogen-containing heterocyclic nucleus of the type found in cyanine dyes and  
 R<sup>7</sup> and R<sup>8</sup> each represent a ring nitrogen substituent of the type found in cyanine dyes.

Z<sup>1</sup> and Z<sup>2</sup> in a preferred form each completes a 5- or 6-membered ring, preferably fused with at least one benzene ring, containing in the ring structure carbon atoms, a single nitrogen atom and, optionally, a sulfur or selenium atom.

Nucleating agents of the type represented by formula (XIV) and their synthesis are disclosed by Baralle et al U.S. Ser. No. 207,814, filed Nov. 17, 1980, commonly assigned and here incorporated by reference (now U.S. Pat. No. 4,306,017).

Still another class of nucleating agents effective in the pH range of from 10 to 13, preferably 10.2 to 12, are diphenylmethane nucleating agents. Such nucleating agents are illustrated by formula (XV) below:



(XV)

wherein  
 Z<sup>1</sup> and Z<sup>2</sup> represent the atoms completing a phenyl nucleus;  
 R<sup>1</sup> represents hydrogen or alkyl of from 1 to 6 carbon atoms; and  
 R<sup>2</sup>, R<sup>3</sup>, and R<sup>4</sup> are independently selected from among hydrogen, halogen, alkyl, hydroxy, alkoxy, aryl, alkaryl, and aralkyl or R<sup>3</sup> and R<sup>4</sup> together form a covalent bond, a divalent chalcogen linkage, or



wherein each alkyl moiety contains from 1 to 6 carbon atoms and each aryl moiety contains 6 to 10 carbon atoms.

Nucleating agents of the type represented by formula (XV) and their synthesis are disclosed by Baralle et al U.S. Ser. No. 205,069, filed Nov. 10, 1980, commonly assigned and here incorporated by reference (now U.S. Pat. No. 4,315,986).

Instead of being incorporated in the photographic element during manufacture, nucleating agents can alternatively or additionally be incorporated in the developer solution. Hydrazine (H<sub>2</sub>N-NH<sub>2</sub>) is an effective nucleating agent which can be incorporated in the developing solution. As an alternative to the use of hydrazine, any of a wide variety of water-soluble hydrazine derivatives can be added to the developing solution. Preferred hydrazine derivatives for use in developing solutions include organic hydrazine compounds of the formula:



where R<sup>1</sup> is an organic radical and each of R<sup>2</sup>, R<sup>3</sup> and R<sup>4</sup> is a hydrogen atom or an organic radical. Organic radicals represented by R<sup>1</sup>, R<sup>2</sup>, R<sup>3</sup> and R<sup>4</sup> include hydrocarbyl groups such as an alkyl group, an aryl group, an aralkyl group, an alkaryl group, and an alicyclic group, as well as hydrocarbyl groups substituted with substituents such as alkoxy groups, carboxy groups, sulfonamido groups, and halogen atoms.

Particularly preferred hydrazine derivatives for incorporation in developing solutions include alkylsulfonamidoaryl hydrazines such as p-(methylsulfonamido)phenylhydrazine and alkylsulfonamidoalkyl aryl hydrazines such as p-(methylsulfonamidomethyl)phenylhydrazine.

The hydrazine and hydrazide derivatives described above are disclosed in Smith et al U.S. Pat. No. 23,410,690, Stauffer et al U.S. Pat. No. 2,419,975, and Hunsberger U.S. Pat. No. 2,892,715. The preferred hydrazines for incorporation in developers are described in Nothnagle U.S. Pat. No. 4,269,929. Another preferred class of nucleating agents that can be incorporated in the developer correspond to formula (I) above, but with the moiety M capable of restricting mobility absent. Nucleating agents of this type are disclosed in Okutsu et al U.S. Pat. No. 4,221,857 and Takada et al U.S. Pat. No. 4,224,401.

#### Silver Imaging

Once core-shell emulsions have been generated by precipitation procedures, washed, and sensitized, as described above, their preparation can be completed by the optional incorporation of nucleating agents, described above, and conventional photographic addenda, and they can be usefully applied to photographic applications requiring a silver image to be produced—e.g., conventional black-and-white photography.

The core-shell emulsion is comprised of a dispersing medium in which the core-shell grains are dispersed. The dispersing medium of the core-shell emulsion layers and other layers of the photographic elements can contain various colloids alone or in combination as vehicles (which include both binders and peptizers).

Preferred peptizers are hydrophilic colloids, which can be employed alone or in combination with hydrophobic materials. Preferred peptizers are gelatin—e.g., alkali-treated gelatin (cattle bone or hide gelatin) and acid-treated gelatin (pigskin gelatin) and gelatin derivatives—e.g., acetylated gelatin, phthalated gelatin, and the like. Useful vehicles are illustrated by those disclosed in *Research Disclosure*, Item 176643, cited above, Section IX, here incorporated by reference. The layers of the photographic elements containing cross-linkable colloids, particularly the gelatin-containing layers, can be hardened by various organic and inorganic hardeners, as illustrated by *Research Disclosure*, Item 17643, cited above, Section X.

Instability which decreases maximum density in direct-positive emulsion coatings can be protected against by incorporation of stabilizers, antifoggants, antikinking agents, latent image stabilizers and similar addenda in the emulsion and contiguous layers prior to coating. A variety of such addenda are disclosed in *Research Disclosure*, Item 17643, cited above, Section VI. Many of the antifoggants which are effective in emulsions can also be used in developers and can be classified under a few general headings, as illustrated by C. E. K. Mees, *The Theory of the Photographic Process*, 2nd Ed., Macmillan, 1954, pp. 677-680.

In some applications improved results can be obtained when the direct-positive emulsions are processed in the presence of certain antifoggants, as disclosed in Stauffer U.S. Pat. No. 2,497,917, here incorporated by reference. Typical useful antifoggants of this type include benzotriazoles, such as benzotriazole, 5-methylbenzotriazole, and 5-ethylbenzotriazole; benzimidazoles such as 5-nitrobenzimidazole; benzothiazoles such as 5-nitrobenzothiazole and 5-methylbenzothiazole; heterocyclic thiones such as 1-methyl-2-tetrazoline-5-thione; triazines such as 2,4-dimethylamino-6-chloro-5-triazine; benzoxazoles such as ethylbenzoxazole; and pyrroles such as 2,5-dimethylpyrrole.

In certain embodiments, good results are obtained when the elements are processed in the presence of high levels of the antifoggants mentioned above. When antifoggants such as benzotriazoles are used, good results can be obtained when the processing solution contains up to 5 grams per liter and preferably 1 to 3 grams per liter; when they are incorporated in the photographic element, concentrations of up to 1,000 mg per mole of silver and preferably concentrations of 100 to 500 mg per mole of silver are employed.

In addition to sensitizers, hardeners, and antifoggants and stabilizers, a variety of other conventional photographic addenda can be present. The specific choice of addenda depends upon the exact nature of the photographic application and is well within the capability of the art. A variety of useful addenda are disclosed in *Research Disclosure*, Item 17632, cited above, here incorporated by reference. Optical brighteners can be introduced, as disclosed by Item 17643 at Section V. Absorbing and scattering materials can be employed in the emulsions of the invention and in separate layers of the photographic elements, as described in Section VIII. Coating aids, as described in Section XI, and plasticizers and lubricants, as described in Section XII, can be present. Antistatic layers, as described in Section XIII, can be present. Methods of addition of addenda are described in Section XIV. Matting agents can be incorporated, as described in Section XVI. Déveloping agents and development modifiers can, if desired, be

incorporated, as described in Sections XX and XXI. The emulsions of the invention, as well as other, conventional silver halide emulsion layers, interlayers, overcoats, and subbing layers, if any, present in the photographic elements can be coated and dried as described in Item 17643, Section XV.

It is specifically contemplated to blend core-shell emulsions of the present invention with each other or with conventional emulsions to satisfy specific emulsion layer requirements. It is specifically contemplated to employ in blending internal latent image-forming grains of similar grain size distribution to minimize migration of addenda between different grain populations. When separate emulsions of similar grain size distribution are employed in combination, their performance can be differentiated by differences in surface sensitization levels, or differences relating to adsorbed nucleating agents, or differences in proportion of internal sensitizers (taught by Atwell et al, cited above). Silverman et al U.S. Ser. No. 320,903, filed concurrently herewith, entitled BLENDED DIRECT-POSITIVE EMULSIONS, PHOTOGRAPHIC ELEMENTS, AND PROCESSES OF USE, commonly assigned and here incorporated by reference (now abandoned in favor of U.S. Ser. No. 418,314, filed Sept. 15, 1962), discloses that the blending of core-shell emulsions in a weight ratio of from 1:5 to 5:1, wherein a first emulsion exhibits a coefficient of variation of less than 20% and a second emulsion has an average grain diameter less than 70% that of the first emulsion, can result in unexpected increase in silver covering power. A speed increase can also be realized, even at reduced coating levels. The ratio of the first emulsion to the second emulsion is preferably 1:3 to 2:1, and the average diameter of the grains of the second emulsion is preferably less than 50%, optimally less than 40% the average diameter of the grains of the first emulsion. The second emulsion can be any conventional internal latent image-forming emulsion, but is preferably substantially free of surface chemical sensitization.

In their simplest form photographic elements according to the present invention employ a single silver halide emulsion layer containing a core-shell emulsion according to the present invention and a photographic support. It is, of course, recognized that more than one silver halide emulsion layer as well as overcoat, subbing, and interlayers can be usefully included. Instead of blending emulsions as described above the same effect can frequently be achieved by coating the emulsions to be blended as separate layers. Coating of separate emulsion layers to achieve exposure latitude is well known in the art, as illustrated by Zelikman and Levi, *Making and Coating Photographic Emulsions*, Focal Press, 1964, pp. 234-238; Wycoff U.S. Pat. No. 3,662,228; and U.K. Pat. No. 923,045. It is further well known in the art that increased photographic speed can be realized when faster and slower silver halide emulsions are coated in separate layers as opposed to blending. Typically the faster emulsion layer is coated to lie nearer the exposing radiation source than the slower emulsion layer. This approach can be extended to three or more superimposed emulsion layers. Such layer arrangements are specifically contemplated in the practice of this invention.

The layers of the photographic elements can be coated on a variety of supports. Typical photographic supports include polymeric film, wood fiber—e.g., paper, metallic sheet and foil, glass and ceramic support-

ing elements provided with one or more subbing layers to enhance the adhesive, antistatic, dimensional, abrasive, hardness, frictional, antihalation and/or other properties of the support surface. Suitable photographic supports are illustrated by *Research Disclosure*, Item 17643, cited above, Section XVII, here incorporated by reference.

Although the emulsion layer or layers are typically coated as continuous layer on supports having opposed planar major surfaces, this need not be the case. The emulsion layers can be coated as laterally displaced layer segments on a planar support surface. When the emulsion layer or layers are segmented, it is preferred to employ a microcellular support. Useful microcellular supports are disclosed by Whitmore Patent Cooperation Treaty published application W080/01614, published Aug. 7, 1980, (Belgian Patent 881,513, Aug. 1, 1980, corresponding), here incorporated by reference. Microcells can range from 1 to 200 microns in width and up to 1000 microns in depth. It is generally preferred that the microcells be at least 4 microns in width and less than 200 microns in depth, with optimum dimensions being about 10 to 100 microns in width and depth for ordinary black-and-white imaging applications—particularly where the photographic image is intended to be enlarged.

The photographic elements of the present invention can be imagewise exposed in any conventional manner. Attention is directed to *Research Disclosure* Item 17643, cited above, Section XVIII, here incorporated by reference. The present invention is particularly advantageous when imagewise exposure is undertaken with electromagnetic radiation within the region of the spectrum in which the spectral sensitizers present exhibit absorption maxima. When the photographic elements are intended to record blue, green, red, or infrared exposures, spectral sensitizer absorbing in the blue, green, red, or infrared portion of the spectrum is present. As noted above, for black-and-white imaging applications it is preferred that the photographic elements be orthochromatically or panchromatically sensitized to permit light to extend sensitivity within the visible spectrum. Radiant energy employed for exposure can be either noncoherent (random phase) or coherent (in phase), produced by lasers. Imagewise exposures at ambient, elevated or reduced temperatures and/or pressures, including high or low intensity exposures, continuous or intermittent exposures, exposure times ranging from minutes to relatively short durations in the millisecond to microsecond range, can be employed within the useful response ranges determined by conventional sensitometric techniques, as illustrated by T. H. James, *The Theory of the Photographic Process*, 4th Ed., Macmillan, 1977, Chapters 4, 6, 17, 18, and 23.

The light-sensitive silver halide contained in the photographic elements can be processed following exposure to form a visible image by associating the silver halide with an aqueous alkaline medium in the presence of a developing agent contained in the medium or the element. Processing formulations and techniques are described in L. F. Mason, *Photographic Processing Chemistry*, Focal Press, London, 1966; *Processing Chemicals and Formulas*, Publication J-1, Eastman Kodak Company, 1973; *Photo-Lab Index*, Morgan and Morgan, Inc., Dobbs Ferry, New York, 1977, and *Neblette's Handbook of Photography and Reprography-Materials, Processes and Systems*, VanNostrand Reinhold Company, 7th Ed., 1977.

Included among the processing methods are web processing, as illustrated by Tregillus et al U.S. Pat. No. 3,179,517; stabilization processing, as illustrated by Herz et al U.S. Pat. No. 3,220,839, Cole U.S. Pat. No. 3,615,511, Shipton et al U.K. Pat. No. 1,258,906 and Haist et al U.S. Pat. No. 3,647,453; monobath processing as described in Haist, *Monobath Manual*, Morgan and Morgan, Inc., 1966, Schuler U.S. Patent 3,240,603, Haist et al U.S. Pat. No. 3,615,513 and 3,628,955 and Price U.S. Pat. No. 3,723,126; infectious development, as illustrated by Milton U.S. Pat. Nos. 3,294,537, 3,600,174, 3,615,519 and 3,615,524, Whiteley U.S. Pat. No. 3,516,830, Drago U.S. Pat. No. 3,615,488, Salesin et al U.S. Pat. No. 3,625,689, Illingsworth U.S. Pat. No. 3,632,340, Salesin U.K. Pat. No. 1,273,030 and U.S. Pat. No. 3,708,303; hardening development, as illustrated by Allen et al U.S. Pat. No. 3,232,761; roller transport processing, as illustrated by Russell et al U.S. Pat. Nos. 3,025,779 and 3,515,556, Masseth U.S. Pat. No. 3,573,914, Taber et al U.S. Pat. No. 3,647,459 and Rees et al U.K. Pat. No. 1,269,268; alkaline vapor processing, as illustrated by *Product Licensing Index*, Vol. 97, May 1972, Item 9711, Goffe et al U.S. Pat. No. 3,816,136 and King U.S. Pat. No. 3,985,564; metal ion development as illustrated by Price, *Photographic Science and Engineering*, Vol. 19, Number 5, 1975, pp. 283-287 and Vought *Research Disclosure*, Vol. 150, October 1976, Item 15034; and surface application processing, as illustrated by Kitze U.S. Pat. No. 3,418,132.

Although development is preferably undertaken in the presence of a nucleating agent, as described above, giving the photographic elements an over-all light exposure either immediately prior to or, preferably, during development can be undertaken as an alternative. When an over-all flash exposure is used, it can be of high intensity and short duration or of lower intensity for a longer duration.

The silver halide developers employed in processing are surface developers. It is understood that the term "surface developer" encompasses those developers which will reveal the surface latent image centers on a silver halide grain, but will not reveal substantial internal latent image centers in an internal latent image-forming emulsion under the conditions generally used to develop a surface-sensitive silver halide emulsion. The surface developers can generally utilize any of the silver halide developing agents or reducing agents, but the developing bath or composition is generally substantially free of a silver halide solvent (such as water-soluble thiocyanates, water-soluble thioethers, thiosulfates, and ammonia) which will disrupt or dissolve the grain to reveal substantial internal image. Low amounts of excess halide are sometimes desirable in the developer or incorporated in the emulsion as halide-releasing compounds, but high amounts of iodide or iodide-releasing compounds are generally avoided to prevent substantial disruption of the grain.

Typical silver halide developing agents which can be used in the developing compositions of this invention include hydroquinones, catechols, aminophenols, 3-pyrazolidinones, ascorbic acid and its derivatives, reductones, phenylenediamines, or combinations thereof. The developing agents can be incorporated in the photographic elements wherein they are brought into contact with the silver halide after imagewise exposure; however, in certain embodiments they are preferably employed in the developing bath.

Once a silver image has been formed in the photographic element, it is conventional practice to fix the undeveloped silver halide. The high aspect ratio tabular grain emulsions are particularly advantageous in allowing fixing to be accomplished in a shorter time period. This allows processing to be accelerated.

#### Dye Imaging

The photographic elements and the techniques described above for producing silver images can be readily adapted to provide a colored image through the use of dyes. In perhaps the simplest approach to obtaining a projectable color image a conventional dye can be incorporated in the support of the photographic element, and silver image formation undertaken as described above. In areas where a silver image is formed the element is rendered substantially incapable of transmitting light therethrough, and in the remaining areas light is transmitted corresponding in color to the color of the support. In this way a colored image can be readily formed. The same effect can also be achieved by using a separate dye filter layer or element with a transparent support element.

The silver halide photographic elements can be used to form dye images therein through the selective destruction or formation of dyes. The photographic elements described above for forming silver images can be used to form dye images by employing developers containing dye image formers, such as color couplers. In this form the developer contains a color-developing agent (e.g., a primary aromatic amine) which in its oxidized form is capable of reacting with the coupler (coupling) to form the image dye. The dye-forming couplers are preferably incorporated in the photographic elements. The dye-forming couplers can be incorporated in different amounts to achieve differing photographic effects. For example, U.K. Pat. No. 923,045 and Kumai et al U.S. Pat. No. 3,843,369 teach limiting the concentration of coupler in relation to the silver coverage to less than normally employed amounts in faster and intermediate speed emulsion layers.

The dye-forming couplers are commonly chosen to form subtractive primary (i.e., yellow, magenta and cyan) image dyes and are nondiffusible, colorless couplers, such as two and four equivalent couplers of the open chain ketomethylene, pyrazolone, pyrazolotriazole, pyrazolobenzimidazole, phenol and naphthol type hydrophobically ballasted for incorporation in high-boiling organic (coupler) solvents. Dye-forming couplers of differing reaction rates in single or separate layers can be employed to achieve desired effects for specific photographic applications.

The dye-forming couplers upon coupling can release photographically useful fragments, such as development inhibitors or accelerators, bleach accelerators, developing agents, silver halide solvents, toners, hardeners, fogging agents, antifoggants, competing couplers, chemical or spectral sensitizers and desensitizers. Development inhibitor-releasing (DIR) couplers are specifically contemplated. Silver halide emulsions which are relatively light insensitive, such as Lippmann emulsions, have been utilized as interlayers and overcoat layers to prevent or control the migration of development inhibitor fragments as described in Shiba et al U.S. Pat. No. 3,892,572. The photographic elements can incorporate colored dye-forming couplers, such as those employed to form integral masks for negative color images. The photographic elements can include

image dye stabilizers. The various couplers and the image dye stabilizers are well known in the art and are illustrated by the various patents cited in *Research Disclosure*, Item 17643, cited above, Section VII, here incorporated by reference.

Dye images can be formed or amplified by processes which employ in combination with a dye-image-generating reducing agent an inert transition metal ion complex oxidizing agent, as illustrated by Bissonette U.S. Pat. Nos. 3,748,138, 3,826,652, 3,862,842 and 3,989,526 and Travis U.S. Pat. No. 3,765,891, and/or a peroxide oxidizing agent, as illustrated by Matejec U.S. Pat. No. 3,674,490, *Research Disclosure*, Vol. 116, December 1973, Item 11660, and Bissonette *Research Disclosure*, Vol. 148, August 1976, Items 14836, 14846 and 14847. The photographic elements can be particularly adapted to form dye images by such processes, as illustrated by Dunn et al U.S. Pat. No. 3,822,129, Bissonette et al U.S. Pat. Nos. 3,834,907 and 3,902,905, Bissonette et al U.S. Pat. No. 3,847,619 and Mowrey U.S. Pat. No. 3,904,413.

It is common practice in forming dye images in silver halide photographic elements to remove the silver which is developed by bleaching. Such removal can be enhanced by incorporation of a bleach accelerator or a precursor thereof in a processing solution or in a layer of the element. In some instances the amount of silver formed by development is small in relation to the amount of dye produced, particularly in dye image amplification, as described above, and silver bleaching is omitted without substantial visual effect. In still other applications the silver image is retained and the dye image is intended to enhance or supplement the density provided by the image silver. In the case of dye enhanced silver imaging it is usually preferred to form a neutral dye or a combination of dyes which together produce a neutral image. Neutral dye-forming couplers useful for this purpose are disclosed by Pupo et al *Research Disclosure*, Vol. 162, October 1977, Item 16226. The enhancement of silver images with dyes in photographic elements intended for thermal processing is disclosed in *Research Disclosure*, Vol. 173, September 1973, Item 17326, and Houle U.S. Pat. No. 4,137,079. It is also possible to form monochromatic or neutral dye images using only dyes, silver being entirely removed from the image-bearing photographic elements by bleaching and fixing, as illustrated by Marchant et al U.S. Pat. No. 3,620,747.

#### Multicolor Photography

The present invention can be employed to produce multicolor photographic images. Generally any conventional multicolor imaging direct-positive photographic element containing at least one core-shell silver halide emulsion layer can be improved merely by substituting a core-shell emulsion according to the present invention.

Significant advantages can be realized by the application of this invention to multicolor photographic elements which produce multicolor images from combinations of subtractive primary imaging dyes. Such photographic elements are comprised of a support and typically at least a triad of super-imposed silver halide emulsion layers for separately recording blue, green, and red light exposures as yellow, magenta, and cyan dye images, respectively. Except as specifically otherwise described, the multicolor photographic elements can

incorporate the features of the photographic elements described previously.

Multicolor photographic elements are often described in terms of color-forming layer units. Most commonly multicolor photographic elements contain three superimposed color-forming layer units each containing at least one silver halide emulsion layer capable of recording exposure to a different third of the spectrum and capable of producing a complementary subtractive primary dye image. Thus, blue, green, and red recording color-forming layer units are used to produce yellow, magenta, and cyan dye images, respectively. Dye imaging materials need not be present in any color-forming layer unit, but can be entirely supplied from processing solutions. When dye imaging materials are incorporated in the photographic element, they can be located in an emulsion layer or in a layer located to receive oxidized developing or electron transfer agent from an adjacent emulsion layer of the same color-forming layer unit.

To prevent migration of oxidized developing or electron transfer agents between color-forming layer units with resultant color degradation, it is common practice to employ scavengers. The scavengers can be located in the emulsion layers themselves, as taught by Yutzy et al U.S. Pat. No. 2,937,086 and/or in interlayers containing scavengers are provided between adjacent color-forming layer units, as illustrated by Weissberger et al U.S. Pat. No. 2,336,327.

Although each color-forming layer unit can contain a single emulsion layer, two, three, or more emulsion layers differing in photographic speed are often incorporated in a single color-forming layer unit. Where the desired layer order arrangement does not permit multiple emulsion layers differing in speed to occur in a single color-forming layer unit, it is common practice to provide multiple (usually two or three) blue, green, and/or red recording color-forming layer units in a single photographic element.

The multicolor photographic elements of this invention can take any convenient form. Any of the six possible layer arrangements of Table 27a, p. 211, disclosed by Gorokhovskii, *Spectral Studies of the Photographic Process*, Focal Press, New York, can be employed. The invention can be better appreciated by reference to certain preferred illustrative forms.

-continued

↓  
G  
IL  
R  
IL  
B

Layer Order Arrangement IV

Exposure  
↓  
FG  
IL  
FR  
IL  
SG  
IL  
SR  
IL  
B

Layer Order Arrangement V

Exposure  
↓  
FG  
IL  
FR  
IL  
FB  
IL  
SG  
IL  
SR  
IL  
SB

30 where

B, G, and R designate blue, green, and red recording color-forming layer units, respectively, of any conventional type;

35 F appearing before the color-forming layer unit B, G, or R indicates that the color-forming layer unit is faster in photographic speed than at least one other color-forming layer unit which records light exposure in the same third of the spectrum in the same Layer Order Arrangement;

40 S appearing before the color-forming layer unit B, G, or R indicates that the color-forming layer unit is slower in photographic speed than at least one other color-forming layer unit which records light exposure in the same third of the spectrum in the same Layer Order Arrangement; and

45 IL designates an interlayer containing a scavenger, and, if needed to protect the green and/or red recording emulsions from blue light exposure, yellow filter material. The placement of green and/or red recording emulsion layers nearer the source of exposing radiation than the blue recording emulsion layer requires the green and/or red recording emulsion layers to be relatively insensitive to blue, such as those containing (1) silver chloride and silver chlorobromide core-shell grains (note Gaspar U.S. Pat. No. 2,344,084) or (2) high aspect ratio tabular grains, as disclosed by the concurrently filed teachings of Evans et al, cited above. Each faster or slower color-

50 forming layer unit can differ in photographic speed from another color-forming layer unit which records light exposure in the same third of the spectrum as a result of its position in the Layer Order Arrangement, its inherent speed properties, or a combination of both.

55 60 65 60 In Layer Order Arrangements I through V, the location of the support is not shown. Following customary practice, the support will in most instances be posi-

Layer Order Arrangement I

Exposure  
↓  
B  
IL  
G  
IL  
R

Layer Order Arrangement II

Exposure  
↓  
FB  
IL  
FG  
IL  
FR  
IL  
SB  
IL  
SG  
IL  
SR

Layer Order Arrangement III

Exposure

tioned farthest from the source of exposing radiation—that is, beneath the layers as shown. If the support is colorless and specularly transmissive—i.e., transparent, it can be located between the exposure source and the indicated layers. Stated more generally, the support can be located between the exposure source and any color-forming layer unit intended to record light to which the support is transparent.

#### Dye Image Transfer

It is possible to construct a dye image transfer film unit according to the present invention capable of producing a monochromatic transferred dye image by locating on a support a single dye-providing layer unit comprised of a core-shell silver halide emulsion layer as described above and at least one dye-image-providing material in the emulsion layer itself or in an adjacent layer of the layer unit. In addition, the dye image transfer film unit is comprised of a dye receiving layer capable of mordanting or otherwise immobilizing dye migrating to it. To produce a transferred dye image the core-shell grain emulsion is imagewise exposed and contacted with an alkaline processing composition with the dye receiving and emulsion layers juxtaposed. In a particularly advantageous application for monochromatic transferred dye images a combination of dye-image-providing materials is employed to provide a neutral transferred dye image. Monochromatic transferred dye images of any hue can be produced, if desired.

Multicolor dye image transfer film units of this invention employ three dye-providing layer units: (1) a cyan-dye-providing layer unit comprised of a red-sensitive silver halide emulsion having associated therewith a cyan-dye-image-providing material, (2) a magenta-dye-providing layer unit comprised of a green-sensitive silver halide emulsion having associated therewith a magenta-dye-image-providing material, and (3) a yellow-dye-providing layer unit comprised of a blue-sensitive silver halide emulsion having associated therewith a yellow-dye-image-providing material. Each of the dye-providing layer units can contain one, two, three, or more separate silver halide emulsion layers as well as the dye-image-providing material, located in the emulsion layers or in one or more separate layers forming part of the dye-providing layer unit. Any one or combination of the emulsion layers can be core-shell silver halide emulsion layers as described above.

Depending upon the dye-image-providing material employed, it can be incorporated in the silver halide emulsion layer or in a separate layer associated with the emulsion layer. The dye-image-providing material can be any of a number known in the art, such as dye-forming couplers, dye developers, and redox dye-releasers, and the particular one employed will depend on the nature of the element or film unit and the type of image desired. Materials useful in diffusion transfer film units contain a dye moiety and a monitoring moiety. The monitoring moiety, in the presence of the alkaline processing solution and as a function of silver halide development, is responsible for a change in mobility of the dye moiety. These dye-image-providing materials can be initially mobile and rendered immobile as a function of silver halide development, as described in Rogers U.S. Pat. No. 2,983,606. Alternatively, they can be initially immobile and rendered mobile, in the presence of an alkaline processing solution, as a function of silver halide development. This latter class of materials in-

clude redox dye-releasing compounds. In such compounds, the monitoring group is a carrier from which the dye is released as a direct function of silver halide development or as an inverse function of silver halide development. Compounds which release dye as a direct function of silver halide development are referred to as negative-working release compounds, while compounds which release dye as an inverse function of silver halide development are referred to as positive-working release compounds. Since the internal latent image-forming emulsions of this invention develop in unexposed areas in the presence of a nucleating agent and a surface developer, positive transferred dye images are produced using negative-working release compounds, and the latter are therefore preferred for use in the practice of this invention.

A preferred class of negative-working release compounds are the ortho or para sulfonamidophenols and naphthols described in Fleckenstein U.S. Pat. No. 4,054,312, Koyama et al U.S. Pat. No. 4,055,428, and Fleckenstein et al U.S. Pat. No. 4,076,529. In these compounds the dye moiety is attached to a sulfonamido group which is ortho or para to the phenolic hydroxy group and is released by hydrolysis after oxidation of the sulfonamido compound during development.

Another preferred class of negative-working release compounds are ballasted dye-forming (chromogenic) or nondye-forming (nonchromogenic) couplers having a mobile dye attached to a coupling-off site. Upon coupling with an oxidized color developing agent, such as a para-phenylenediamine, the mobile dye is displaced so that it can transfer to a receiver. The use of such negative-working dye image providing compounds is illustrated by Whitmore et al U.S. Pat. No. 3,227,550, Whitmore U.S. Pat. No. 3,227,552, and Fujiwhara et al U.K. Pat. No. 1,445,797, the disclosures of which are here incorporated by reference.

Since the silver halide emulsions employed in the image transfer film units of the present invention are positive-working, the use of positive-working release compounds will produce negative transferred dye images. Useful positive-working release compounds are nitrobenzene and quinone compounds described in Chasman et al U.S. Pat. No. 4,139,379, the hydroquinones described in Fields et al U.S. Pat. No. 3,980,479 and the benzisoxazolone compounds described in Hinshaw et al U.S. Pat. No. 4,199,354.

Further details regarding the above release compounds, the manner in which they function, and the procedures by which they can be prepared are contained in the patents referred to above, the disclosures of which are incorporated herein by reference.

Any material can be employed as the dye receiving layer in the film units of this invention as long as it will mordant or otherwise immobilize the dye which diffuses to it. The optimum material chosen will, of course, depend upon the specific dye or dyes to be mordanted. The dye receiving layer can also contain ultraviolet absorbers to protect the dye image from fading due to ultraviolet light, brighteners, and similar materials to protect or enhance the dye image. A polyvalent metal, preferably immobilized by association with a polymer, can be placed in or adjacent in the receiving layer to chelate the transferred image dye, as taught by Archie et al U.S. Pat. No. 4,239,849 and Myers et al U.S. Pat. No. 4,241,163. Useful dye receiving layers and materials for their fabrication are disclosed in *Research Disclosure*

Item 15162, cited above, and Morgan et al European Patent Publication 14,584.

The alkaline processing composition employed in the dye image transfer film units can be an aqueous solution of an alkaline material, such as an alkali metal hydroxide or carbonate (e.g., sodium hydroxide or sodium carbonate) or an amine (e.g., diethylamine). Preferably the alkaline composition has a pH in excess of 11. Suitable materials for use in such compositions are disclosed in *Research Disclosure*, Item 15162, cited above.

A developing agent is preferably contained in the alkaline processing composition, although it can be contained in a separate solution or process sheet, or it can be incorporated in any processing solution penetrable layer of the film unit. When the developing agent is separate from the alkaline processing composition, the alkaline composition serves to activate the developing agent and provide a medium in which the developing agent can contact and develop silver halide.

A variety of silver halide developing agents can be used in processing the film units of this invention. The choice of an optimum developing agent will depend on the type or film unit with which it is used and the particular dye image-providing material employed. Suitable developing agents can be selected from such compounds as hydroquinone, aminophenols (e.g., N-methylaminophenol), 1-phenyl-3-pyrazolidinone, 1-phenyl-4,4-dimethyl-3-pyrazolidinone, 1-phenyl-4-methyl-4-hydroxymethyl-3-pyrazolidinone, and N,N,N',N'-tetramethyl-p-phenylenediamine. The non-chromogenic developers in this list are preferred for use in dye transfer film units, since they have a reduced propensity to stain dye image-receiving layers.

The image transfer film units of this invention can employ any layer order arrangement heretofore known to be useful in conventional image transfer film units having one or more radiation-sensitive silver halide emulsion layers. The following specific layer order arrangements, are merely illustrative, many other arrangements being additionally contemplated:

---

Image Transfer Film Unit I

---

A Peel-Apart Dye Image Transfer Film Unit  
 Reflective Support  
 Dye Receiving Layer  
 Imagewise Exposure  
 ↓  
 Core-Shell Silver Halide Emulsion Layer  
 With Dye-Image-Providing Material  
 Support

---

Image Transfer Film Unit I illustrative of a conventional peel-apart image transfer film unit. Upon imagewise exposure, the positive-working core-shell silver halide emulsion layer produces a developable latent image at centers located on the interior of exposed grains. The dye receiving layer is laminated and an alkaline processing composition, not shown, is released between the dye receiving layer and emulsion layer following exposure. Upon contact with the alkaline processing composition development of the core-shell silver halide grains bearing internal latent image centers occurs much more slowly than the development of silver halide grains which do not contain internal latent image centers. Using a negative-working dye-image-providing material dye is released in those areas in which silver development occurs and migrates to the dye receiving layer where it is held in place by a mordant. A positive transferred dye image is produced in

the dye receiving layer. Processing is terminated by peeling the reflective support having the dye receiving layer coated thereon from the remainder of the image transfer film unit.

---

Image Transfer Film Unit II

---

An Integral Monochromatic Dye Image Transfer Film Unit  
 View

↓  
 Transparent Support

Dye Receiving Layer

Reflective Layer

Opaque Layer

Core-shell Silver Halide Emulsion Layer

With Dye-Image Providing Material

Alkaline Processing Solution + Opacifier

Timing Layer

Neutralizing Layer

Transparent Support

↑  
 Imagewise Exposure

---

Initially the alkaline processing composition containing opacifier is not present in the location shown. Therefore, upon imagewise exposure light strikes the core-shell silver halide emulsion layer. This produces a latent image corresponding to light-struck areas of the emulsion layer. To initiate processing the alkaline processing composition is placed in the position shown. Usually, but not necessarily, the image transfer film unit is removed from the camera in which it is exposed immediately following placement of the alkaline processing composition and opacifier. The opacifier and opaque layer together prevent further exposure of the emulsion layer. Upon development, a mobile dye or dye precursor is released from the emulsion layer. The mobile dye or dye precursor penetrates the opaque layer and the reflective layer and is mordanted or otherwise immobilized in the dye receiving layer to permit viewing through the uppermost transparent support. Processing is terminated by the timing and neutralizing layers.

---

Image Transfer Film Unit III

---

An Integral Multicolor Dye Image Transfer Film Unit  
 Imagewise Exposure

↓  
 Transparent Support

Neutralizing Layer

Timing Layer

Alkaline Processing Composition + Opacifier

Transparent Overcoat

Blue-sensitive Core-shell Silver

Halide Emulsion Layer

Yellow Dye-Image-Providing Material Layer

Interlayer With Scavenger

Green-sensitive Core-shell Silver

Halide Emulsion Layer

Magenta Dye-Image-Providing Material Layer

Interlayer With Scavenger

Red-sensitive Core-shell Silver

Halide Emulsion Layer

Cyan Dye-Image-Providing Material Layer

Opaque Layer

Reflective Layer

Dye Receiving Layer

Transparent Support

↑  
 View

---

Image Transfer Film Unit III is essentially similar to Image Transfer Film Unit II, but is modified to contain

three separate dye-providing layer units, each comprised of one core-shell grain silver halide emulsion layer and one dye-image-providing material layer, instead of the single dye-image-providing material containing core-shell grain silver halide emulsion layer of Image Transfer Film Unit II. (Whether or not the dye-image-providing material is placed in the emulsion layer itself or in an adjacent layer in Image Transfer Film Units II and III is a matter of choice, either arrangement being feasible).

To prevent color contamination of adjacent dye-providing layer units, an interlayer containing a scavenger is positioned between dye-providing layer units. The use of scavengers in interlayers and/or in the dye-providing layer units themselves is contemplated. In some instances reductions in minimum edge densities can also be realized by incorporating a negative-working silver halide emulsion in the interlayers. In a modification of Image Transfer Film Unit III it is possible to eliminate the interlayers.

#### Image Transfer Film Unit IV

An Integral Multicolor Dye Image Transfer Film Unit  
Opaque Support  
Yellow Dye-Image-Providing Material Layer  
Blue-sensitive Core-shell Silver  
Halide Emulsion Layer  
Interlayer With Scavenger  
Cyan Dye-Image-Providing Material Layer  
Red-sensitive Core-shell Silver  
Halide Emulsion Layer  
Interlayer With Scavenger  
Magenta Dye-Image-Providing Material Layer  
Green-sensitive Core-shell Silver  
Halide Emulsion Layer  
Transparent Overcoat  
Alkaline Processing Composition With  
Reflective Material and Indicator Dye  
Dye Receiving Layer  
Timing Layer  
Neutralizing Layer  
Transparent Support  
↑  
View and Imagewise Exposure

In Image Transfer Film Unit IV during image-wise exposure the alkaline processing composition containing the reflective material and indicator dye is not in the position shown, but is released to the position shown after exposure to permit processing. The indicator dye exhibits a high density at the elevated levels of pH under which processing occurs. It thereby protects the silver halide emulsion layers from further exposure if the film unit is removed from a camera during processing. Once the neutralizing layer reduces the pH within the film unit to terminate processing, the indicator dye reverts to an essentially colorless form. The alkaline processing composition also contains an opaque reflective material, which provides a white background for viewing the transferred dye image after processing and prevents additional exposure.

Although the invention has been particularly described with reference to certain preferred layer order arrangements, it is appreciated that the core-shell silver halide emulsions need not always be present as planar, uninterrupted layers. Rather than being continuous, the layers can be subdivided into discrete laterally displaced portions or segments. In multicolor image transfer film units the layers need not be superimposed, but can be present in the form of interlaid layer segments. It is specifically contemplated to employ core-shell silver

halide emulsions as herein disclosed in microcellular image transfer film unit arrangements, such as disclosed by Whitmore Patent Cooperation Treaty published application W080/01614, published Aug. 7, 1980, here incorporated by reference. The present invention is also fully applicable to microcellular image transfer film units containing microcells which are improvements on Whitmore, such as Gilmour U.S. Ser. No. 192,976, filed Oct. 1, 1980, titled AN IMPROVEMENT IN THE FABRICATION OF ARRAYS CONTAINING INTERLAID PATTERNS OF MICROCELLS (now abandoned in favor of U.S. Ser. No. 375,423, filed May 6, 1982); Blazey et al U.S. Ser. No. 193,065, filed Oct. 2, 1980, titled PLURAL IMAGING COMPONENT MICROCELLULAR ARRAYS, PROCESSES FOR THEIR FABRICATION AND ELECTROPHOTOGRAPHIC COMPOSITIONS (now U.S. Pat. No. 4,307,165); and Gilmour et al U.S. Ser. No. 196,947, filed Oct. 14, 1980, entitled ELEMENTS CONTAINING ORDERED WALL ARRAYS AND PROCESS FOR THEIR FABRICATION (now abandoned in favor of U.S. Ser. No. 293,080, filed Aug. 17, 1981), the disclosures of which are here incorporated by reference.

Image transfer film units and features thereof useful in the practice of this invention are further illustrated by *Research Disclosure*, Item 15162, cited above and here incorporated by reference.

The invention can be better appreciated by reference to the following examples:

#### EXAMPLE 1

A 0.41  $\mu\text{m}$  AgCl emulsion was prepared by a double-jet precipitation technique and chemically sensitized with 1.2 mg  $\text{Na}_2\text{S}_2\text{O}_3 \cdot 5\text{H}_2\text{O}$ /mole Ag and 1.8 mg  $\text{KAuCl}_4$ /mole Ag for 30 minutes at 70° C. The emulsion was divided into two parts, A and B. Part A was precipitated with additional AgCl to yield a 0.65  $\mu\text{m}$  core-shell AgCl emulsion. To Part B, 4 mg  $\text{CdCl}_2$ /mole silver was added and the emulsion was further precipitated with AgCl to yield a 0.59  $\mu\text{m}$  core-shell AgCl emulsion. Both emulsions were then chemically sensitized with 2.0 mg  $\text{Au}_2\text{S}$ /mole silver for 10 minutes at 60° C. The emulsions were coated on a polyester film support at 1.07 g/ $\text{m}^2$  silver and 2.15 g/ $\text{m}^2$  gelatin. The coatings also contained 1.07 g/ $\text{m}^2$  cyan coupler A, and were overcoated with 1.07 g/ $\text{m}^2$  gelatin and hardened with 1% bis(vinylsulfonylmethyl) ether by weight based on total gelatin content. The coatings were exposed for 1/5" through a 0-6.0 step tablet to a 500 W, 3000° K. tungsten light source and processed for 2 minutes at 33.4° C. in a p-phenylenediamine color developer solution containing 8 mg/l benzotriazole and 50 mg/l formyl-4-methyl-phenylhydrazine as the fogging agent.

Sensitometric results are given in Table I.

TABLE I

Effect of Cadmium Chloride in Shell of Core-Shell Internal-Image AgCl Emulsion

| Coating    | $\text{CdCl}_2$ | Reversal  |           | $\Delta \log E^*$<br>Reversal-Surface<br>Negative |
|------------|-----------------|-----------|-----------|---------------------------------------------------|
|            |                 | $D_{max}$ | $D_{min}$ |                                                   |
| Emulsion A | None            | 3.58      | .34       | .53                                               |
| Emulsion B | Shell           | 3.62      | .08       | 1.05                                              |

\* $\Delta \log E$  between reversal image and the surface negative image. Relative  $\log E$  values taken at 0.10 density unit above  $D_{min}$ . E is exposure in meter-candle-seconds.

As demonstrated in Table I, the use of cadmium chloride in concentrations of 4 mg/Ag mole ( $2.2 \times 10^{-5}$  mole/Ag mole) during the shelling stage of precipitation lowers the minimum density ( $D_{min}$ ). In addition, it extends by 0.52 log E the overexposure required to encounter rereversal.

### EXAMPLE 2

This example illustrates the application of the invention to high aspect ratio tubular grain core-shell emulsions of the type which form the subject matter of the concurrently filed patent application of Evans et al, cited above.

#### Emulsion A: Core Tabular AgBrI Emulsion

A AgI seed grain emulsion was prepared by a double-jet precipitation technique at pH 2.85 and 35° C. To prepare 0.125 moles of emulsion 5.0 M silver nitrate and 5.0 M sodium iodide solutions were added over a period of 3.5 minutes to a reaction vessel containing 60 grams of deionized bone gelatin dissolved in 2.5 liters of water. The resulting silver iodide emulsion had a mean grain diameter of 0.027  $\mu$ m and the crystals were of hexagonal bipyramidal structure.

Then 1.75 moles of silver bromide was precipitated onto  $2.4 \times 10^{-3}$  mole of the silver iodide seed grains by a double-jet technique. 4.0 M silver nitrate and 4.0 M sodium bromide reagents were added over a 15 minute period at 80° C. using accelerated flow (6.0X from start to finish). The pBr was maintained at 1.3 during the first 5 minutes, adjusted to a pBr of 2.2 over the next 3 minutes, and maintained at 2.2 for the remainder of the precipitation.

The resulting tabular AgBrI crystals had a mean grain diameter of 1.0  $\mu$ m, an average thickness of 0.08  $\mu$ m, and an average aspect ratio of 12.5:1 and account for greater than 90 percent of the total projected surface area of the silver halide grains.

Emulsion A was then chemically sensitized with 1.9 mg/Ag mole sodium thiosulfate pentahydrate and 2.9 mg/Ag mole potassium tetrachloroaurate for 30 minutes at 80° C.

#### Control Emulsion B: Core/Shell Tabular AgBrI Emulsion

The chemically sensitized Emulsion A (0.22 mole) was placed in a reaction vessel at pBr 1.7 at 80° C. Then onto Emulsion A, 5.78 moles of silver bromide were precipitated by a double-jet addition technique. 4.0 M silver nitrate and 4.0 M sodium bromide solutions were added in an accelerated flow (4.0X from start to finish) over a period of 46.5 minutes while maintaining a pBr of 1.7. The resulting AgBrI crystals had a mean grain diameter of 3.0  $\mu$ m, an average thickness of 0.25  $\mu$ m, and average aspect ratio of 12:1.

Emulsion B was chemically sensitized with 1.0 mg/Ag mole sodium thiosulfate pentahydrate for 40 minutes at 74° C. and red spectrally sensitized with 250 mg/Ag mole anhydro-5,5'-dichloro-9-ethyl-3,3'-bis(3-sulfobutyl)thiacarbocyanine hydroxide.

#### Emulsion C: Cadmium Doped Tabular AgBrI Internal Latent Image-Forming Emulsion

Emulsion C was prepared the same as Emulsion B with the exception that at 8 minutes into the shelling stage of the core/shell precipitation cadmium bromide was added at 0.05 mole percent (based on the moles of silver in the shell).

An integral imaging receiver (IIR) of the following layer order arrangement was prepared: Coverages are

in (g/m<sup>2</sup>) or [mg/Ag mole]. Chemical structures are shown in the Appendix below.

|          |                                                                                                                                     |
|----------|-------------------------------------------------------------------------------------------------------------------------------------|
| Layer 8: | Overcoat layer: Scavenger I (0.11), gelatin (0.89), Bis(vinylsulfonylmethyl)ether hardener at 1 percent of the total gelatin weight |
| Layer 7: | Red-sensitive silver halide layer: Emulsion C (1.34 Ag), Nucleating Agent II [2.0], Scavenger III [4000], gelatin (1.34)            |
| Layer 6: | Gel (0.43) interlayer                                                                                                               |
| Layer 5: | Interlayer: Titanium dioxide (0.81), gelatin (0.65)                                                                                 |
| Layer 4: | Cyan dye-releaser layer: RDR IV (0.43), gelatin (0.65)                                                                              |
| Layer 3: | Opaque layer: Carbon (1.9), RDR V (0.02), Scavenger III (0.03), gelatin (1.2)                                                       |
| Layer 2: | Reflecting layer: Titanium dioxide (22.0), gelatin (3.4)                                                                            |
| Layer 1: | Receiving layer: Mordant VI (4.8), gelatin (2.3)                                                                                    |

The layers were coated on a clear polyester support in the order of numbering.

A control integral imaging receiver of the same layer order arrangement was prepared as above except Layer 7 had Emulsion B.

The following processing pod composition was employed in both units:

|                                                            |           |
|------------------------------------------------------------|-----------|
| Potassium hydroxide                                        | 46.8 g/l  |
| 4-Methyl-4-hydroxymethyl-1- <i>p</i> -tolyl-3-pyrazolidone | 15.0 g/l  |
| 5-Methylbenzotriazole                                      | 5.0 g/l   |
| Carboxymethylcellulose                                     | 46.0 g/l  |
| Potassium fluoride                                         | 10.0 g/l  |
| Tamol SN @ dispersant                                      | 6.4 g/l   |
| Potassium sulfite (anhydrous)                              | 3.0 g/l   |
| 1,4-Cyclohexanedimethanol                                  | 3.0 g/l   |
| Carbon                                                     | 191.0 g/l |

Two cover sheets of the following structure were prepared:

Layer 2: Timing layer: 1:1 physical mixture of the following two polymers coated at 3.2 g/m<sup>2</sup>.

Poly(acrylonitrile-co-vinylidene chloride-co-acrylic acid) at a weight ratio of 14:79:7 (isolated as a latex, dried and dispersed in an organic solvent). A carboxy ester lactone was formed by cyclization of a vinyl acetate-maleic anhydride copolymer in the presence of 1-butanol to produce a partial butyl ester with a weight ratio of acid to butyl ester of 15:85 (See Abel U.S. Pat. No. 4,229,516). This layer also contains t-butylhydroquinone monoacetate at 0.043 g/m<sup>2</sup> as a competitor and 5-(2-cyanoethylthio)-1-phenyltetrazole at 0.043 g/m<sup>2</sup> as a blocked inhibitor.

Layer 1: Acid layer: Poly(n-butyl acrylate-co-acrylic acid) 30:70 weight ratio equivalent to 140 meq acid/m<sup>2</sup>. The layers were coated on a clear polyester support in the order of numbering.

The above image transfer film units including the processing composition and cover sheet were used in the following manner:

Each multicolor photosensitive integral imaging receiver was exposed for 1/100 second in a sensitometer through a step tablet to 5000° K. illumination (daylight balance-neutral), then processed at room temperature using a viscous processing composition contained in a pod. The processing composition was spread between

the IIR and the transparent cover sheet using a pair of juxtaposed rollers to provide a processing gap of about 65  $\mu\text{m}$ .

After a period of more than one hour the red density of the stepped image was read. The red minimum density ( $D_{min}$ ) and maximum density ( $D_{max}$ ) values were read from the above produced sensitometric curve. Threshold reversal speeds are read at 0.3 density below  $D_{max}$ , the reversal/rereversal separation is read at 0.7 density. A difference of 30 relative speed units equals  $0.30 \log E$ .

The data below show that the cadmium doped emulsion is  $0.20 \log E$  faster and has a net speed reversal/-rereversal separation of  $0.37 \log E$  more than does the corresponding emulsion free of cadmium doping. It is highly desirable that the reversal speed becomes faster and the rereversal speed slower.

| Emulsion              | Relative<br>Reversal<br>Speed (D = 0.7) | Relative<br>Rereversal<br>Speed (D = 0.7) | Δ          |
|-----------------------|-----------------------------------------|-------------------------------------------|------------|
| B (non CdII<br>doped) | 272                                     | 77                                        | 195        |
| C (CdII doped)        | 292                                     | 60                                        | <u>232</u> |
|                       |                                         | (Net gain                                 | 37)        |

Experimental results have also shown that the surface negative image can be significantly reduced if the shell portion of the tabular grain emulsion is doped with either lead (II) or erbium (III).

## APPENDIX

### Scavenger I



### Nucleating Agent II



### Scavenger Hunt



Cyan RDR IV

## APPENDIX-continued



Cyan RDR V



Mémoires VI

poly(styrene-co-1-vinylimidazole-co-3-benzyl-1-vinylimidazolium chloride) (weight ratio approx. 50:40:10)

The invention has been described in detail with particular reference to preferred embodiments thereof, but it will be understood that variations and modifications can be effected within the spirit and scope of the invention.

What is claimed is:

1. A radiation-sensitive emulsion particularly adapted to forming a direct-positive image comprised of a dispersing medium and silver halide grains capable of forming an internal latent image, said silver halide grains being comprised of a sensitized core and a shell, and said shell incorporating in an amount sufficient to reduce rereversal one or more polyvalent metal ions chosen from the group consisting of manganese, copper, zinc, cadmium, lead, bismuth, and lanthanides, said emulsion when coated on a transparent film support at a silver coverage of 4 grams per square meter, exposed to a 500 watt tungsten lamp for times ranging from 0.01 to 1 second at a distance of 0.6 meter, developed for 5 minutes at 20° C. in Developer Y below, fixed, washed, and dried, having a maximum density at least five times the maximum density of an identical test portion which has been exposed in the same way and developed for 6 minutes at 20° C. in Developer X below, fixed, washed, and dried:

|                                |      | Grams |
|--------------------------------|------|-------|
| <u>Developer X</u>             |      |       |
| N-methyl-p-aminophenol sulfate | 2.5  | 5     |
| Ascorbic acid                  | 10.0 |       |
| Potassium metaborate           | 35.0 |       |
| Potassium bromide              | 1.0  |       |
| Water to 1 liter               |      |       |
| <u>Developer Y</u>             |      |       |
| N-methyl-p-aminophenol sulfate | 2.0  | 10    |
| Sodium sulfite, desiccated     | 90.0 |       |
| Hydroquinone                   | 8.0  |       |
| Sodium carbonate, monohydrate  | 52.5 |       |
| Potassium bromide              | 5.0  |       |
| Potassium iodide               | 0.5  |       |
| Water to 1 liter.              |      | 15    |

2. A radiation-sensitive emulsion according to claim 1 wherein said silver halide grains are comprised of chloride.

3. A radiation-sensitive emulsion according to claim 2 wherein at least said shells of said silver halide grains contain at least 80 mole percent chloride, based on total halide.

4. A radiation-sensitive emulsion according to claim 1 wherein said silver halide grains are comprised of bromide.

5. A radiation-sensitive emulsion according to claim 4 wherein said silver halide grains are additionally comprised of iodide.

6. A radiation-sensitive emulsion according to claim 1 wherein said dispersing medium is comprised of a peptizer.

7. A radiation-sensitive emulsion according to claim 6 wherein said peptizer is gelatin or a gelatin derivative.

8. A radiation-sensitive emulsion according to claim 1 additionally including a nucleating agent incorporated therein.

9. A radiation-sensitive emulsion according to claim 8 wherein said nucleating agent is chosen from the class consisting of aromatic hydrazide nucleating agents, N-substituted cycloammonium quaternary salt nucleating agents, and mixtures thereof.

10. A radiation-sensitive emulsion according to claim 8 wherein said nucleating agent is a hydrazide of the formula



wherein

D is an acyl group;

φ is a phenylene or a halo-, alkyl-, or alkoxy-substituted phenylene group; and

M is a moiety capable of restricting mobility.

11. A radiation-sensitive emulsion particularly adapted to forming a direct-positive image comprised of a nucleating agent, gelatin or a gelatin-derived peptizer, silver halide grains sensitized with at least one of sulfur, selenium, and gold, and capable of forming an internal latent image, said silver halide grains being comprised of a core and a shell, and said shell incorporating a divalent or trivalent metal cationic dopant in a concentration of from about  $10^{-3}$  to  $10^{-7}$  mole per mole of silver chosen from the group consisting of manganese, copper, zinc, cadmium, lead, bismuth, and lanthanides, said

emulsion when coated on a transparent film support at a silver coverage of 4 grams per square meter, exposed to a 500 watt tungsten lamp for times ranging from 0.01 to 1 second at a distance of 0.6 meter, developed for 5 minutes at 20° C. in Developer Y below, fixed, washed, and dried, having a maximum density at least five times the maximum density of an identical test portion which has been exposed in the same way and developed for 6 minutes at 20° C. in Developer X below, fixed, washed, and dried:

|                                |      | Grams |
|--------------------------------|------|-------|
| <u>Developer X</u>             |      |       |
| N-methyl-p-aminophenol sulfate | 2.5  |       |
| Ascorbic acid                  | 10.0 |       |
| Potassium metaborate           | 35.0 |       |
| Potassium bromide              | 1.0  |       |
| Water to 1 liter               |      |       |
| <u>Developer Y</u>             |      |       |
| N-methyl-p-aminophenol sulfate | 2.0  |       |
| Sodium sulfite, desiccated     | 90.0 |       |
| Hydroquinone                   | 8.0  |       |
| Sodium carbonate, monohydrate  | 52.5 |       |
| Potassium bromide              | 5.0  |       |
| Potassium iodide               | 0.5  |       |
| Water to 1 liter.              |      |       |

12. A radiation-sensitive emulsion according to claim 11 wherein said dopant is chosen from Group IIB of the periodic table of elements.

13. A radiation-sensitive emulsion according to claim 11 wherein said dopant is cadmium.

14. A radiation-sensitive emulsion according to claim 11 wherein said dopant is lead.

15. A radiation-sensitive emulsion according to claim 11 wherein said dopant is erbium.

16. A radiation-sensitive emulsion according to claim 11 wherein said dopant is present in a concentration of from  $5 \times 10^{-4}$  to  $10^{-6}$  mole per mole of silver.

17. A radiation-sensitive emulsion according to claim 11 wherein said nucleating agent is a phenylhydrazide of the formula



wherein

R is hydrogen or an alkyl, cycloalkyl, haloalkyl, alkoxyalkyl, or phenylalkyl substituent or a phenyl nucleus having a Hammett sigma-value-derived electron-withdrawing characteristic more positive than -0.30;

R<sup>1</sup> is a phenylene or alkyl, halo-, or alkoxy-substituted phenylene group;

R<sup>2</sup> is hydrogen, benzyl, alkoxybenzyl, halobenzyl, or alkylbenzyl;

R<sup>3</sup> is a alkyl, haloalkyl, alkoxyalkyl, or phenylalkyl substituent having from 1 to 18 carbon atoms, a cycloalkyl substituent, a phenyl nucleus having a Hammett sigma value-derived electron-withdrawing characteristic less positive than +0.50, or naphthyl, and

R<sup>4</sup> is hydrogen or independently selected from among the same substituents as R<sup>3</sup>, or

$R^3$  and  $R^4$  together form a heterocyclic nucleus forming a 5- or 6-membered ring, wherein the ring atoms are chosen from the class consisting of nitrogen, carbon, oxygen, sulfur, and selenium atoms; the alkyl moieties, except as otherwise noted, in each instance include from 1 to 6 carbon atoms and the cycloalkyl moieties have from 3 to 10 carbon atoms and at least one of  $R^2$  and  $R^3$  must be hydrogen.

18. A radiation-sensitive emulsion according to claim 11 wherein said nucleating agent is a hydrazide or hydrazone of the formula



15

wherein

$T$  is a phenyl or naphthyl substituent;

$T^1$  is an acyl radical; and

$T^2$  is an alkylidene substituent having from 1 to 22 carbon atoms.

20

19. A radiation-sensitive emulsion particularly adapted to forming a direct-positive dye image comprised of

a dye image former,

25

a nucleating agent,

silver halide grains sensitized with at least one of sulfur, selenium, and gold capable of forming an internal latent image,

said silver halide grains being comprised of a core and a shell, and

said shell incorporating divalent cadmium in a concentration of from about  $5 \times 10^{-4}$  to  $10^{-6}$  mole per mole of silver, said emulsion when coated on a transparent film support at a siver coverage of 4

35

grams per square meter, exposed to a 500 watt tungsten lamp for times ranging from 0.01 to 1 second at a distance of 0.6 meter, developed for 5 minutes at 20° C. in Developer Y below, fixed, washed, and dried, having a maximum density at least five times the maximum density of an identical test portion which has been exposed in the same way and developed for 6 minutes at 20° C. in Developer X below, fixed, washed, and dried:

40

|                                | Grams |
|--------------------------------|-------|
| <u>Developer X</u>             |       |
| N-methyl-p-aminophenol sulfate | 2.5   |
| Ascorbic acid                  | 10.0  |
| Potassium metaborate           | 35.0  |
| Potassium bromide              | 1.0   |
| Water to 1 liter               |       |
| <u>Developer Y</u>             |       |
| N-methyl-p-aminophenol sulfate | 2.0   |
| Sodium sulfite, desiccated     | 90.0  |
| Hydroquinone                   | 8.0   |
| Sodium carbonate, monohydrate  | 52.5  |
| Potassium bromide              | 5.0   |
| Potassium iodide               | 0.5   |
| Water to 1 liter.              |       |

45

20. In a direct-positive photographic element comprised of a support and at least one radiation-sensitive emulsion layer, the improvement wherein said emulsion layer is comprised of an emulsion according to claim 1, 2, 3, 4, 5, 6, 7, 8, 9, 10, 11, 12, 13, 14, 15, 16, 17, 18 or 19.

65

21. Processing in a surface developer an imagewise exposed photographic element according to claim 20 (a) in the presence of a nucleating agent or

(b) with light flashing of the exposed photographic element during processing.

22. In a multicolor direct-positive photographic element comprised of a support and, located thereon, emulsion layers for separately recording blue, green, and red light each comprised of a dispersing medium, internal latent image-forming core-shell silver halide grains, and a nucleating agent, said emulsion when coated on a transparent film support at a siver coverage of 4 grams per square meter, exposed to a 500 watt tungsten lamp for times ranging from 0.01 to 1 second at a distance of 0.6 meter, developed for 5 minutes at 20° C. in Developer Y below, fixed, washed, and dried, having a maximum density at least five times the maximum density of an identical test portion which has been exposed in the same way and developed for 6 minutes at 20° C. in Developer X below, fixed, washed, and dried:

|                                | Grams |
|--------------------------------|-------|
| <u>Developer X</u>             |       |
| N-methyl-p-aminophenol sulfate | 2.5   |
| Ascorbic acid                  | 10.0  |
| Potassium metaborate           | 35.0  |
| Potassium bromide              | 1.0   |
| Water to 1 liter               |       |
| <u>Developer Y</u>             |       |
| N-methyl-p-aminophenol sulfate | 2.0   |
| Sodium sulfite, desiccated     | 90.0  |
| Hydroquinone                   | 8.0   |
| Sodium carbonate, monohydrate  | 52.5  |
| Potassium bromide              | 5.0   |
| Potassium iodide               | 0.5   |
| Water to 1 liter.              |       |

the improvement comprising said core-shell silver halide grains in at least one of said emulsion layers being sensitized with at least one of sulfur, selenium, and gold and containing a shell portion incorporating in an amount sufficient to reduce rereversal one or more polyvalent metal ions chosen from the group consisting of manganese, copper, zinc, cadmium, lead, bismuth, and lanthanides.

23. In a photographic image transfer film unit comprising

a support,

at least one emulsion layer located on said support containing a dispersing medium, radiation-sensitive core-shell internal latent image-forming silver halide grains, and a nucleating agent, said emulsion when coated on a transparent film support at a siver coverage of 4 grams per square meter, exposed to a 500 watt tungsten lamp for times ranging from 0.01 to 1 second at a distance of 0.6 meter, developed for 5 minutes at 20° C. in Developer Y below, fixed, washed, and dried, having a maximum density at least five times the maximum density of an identical test portion which has been exposed in the same way and developed for 6 minutes at 20° C. in Developer X below, fixed, washed, and dried:

|                                | Grams |
|--------------------------------|-------|
| <u>Developer X</u>             |       |
| N-methyl-p-aminophenol sulfate | 2.5   |
| Ascorbic acid                  | 10.0  |

-continued

|                                | Grams |
|--------------------------------|-------|
| Potassium metaborate           | 35.0  |
| Potassium bromide              | 1.0   |
| Water to 1 liter               |       |
| <u>Developer Y</u>             |       |
| N-methyl-p-aminophenol sulfate | 2.0   |
| Sodium sulfite, desiccated     | 90.0  |
| Hydroquinone                   | 8.0   |
| Sodium carbonate, monohydrate  | 52.5  |
| Potassium bromide              | 5.0   |
| Potassium iodide               | 0.5   |
| Water to 1 liter.              |       |

a dye-image-providing material present in said emulsion layer or a layer adjacent thereto, and

a receiving layer for providing a viewable transferred dye image following imagewise exposure and processing of said emulsion layer,

the improvement comprising, said core-shell silver halide grains present in at least one emulsion layer being sensitized with at least one of sulfur, selenium, and gold and containing a shell portion incorporating in an amount sufficient to reduce rereversal one or more polyvalent metal ions chosen from the group consisting of manganese, copper, zinc, cadmium, lead, bismuth, and lanthanides.

24. In the photographic element or film unit of claim 22 or 23 the further improvement in which said shell portion includes at least one of cadmium (II), lead (II) and erbium (III) in a concentration of from  $5 \times 10^{-4}$  to  $10^{-6}$  mole per mole of silver.

\* \* \* \* \*

20

25

30

35

40

45

50

55

60

65

UNITED STATES PATENT AND TRADEMARK OFFICE  
CERTIFICATE OF CORRECTION

PATENT NO. : 4,395,478

DATED : July 26, 1983

INVENTOR(S) : Harry A. Hoyen

It is certified that error appears in the above-identified patent and that said Letters Patent  
are hereby corrected as shown below:

Title page, second column under U.S. PATENT DOCUMENTS, after  
the second line thereof,

|             |         |                |
|-------------|---------|----------------|
| --2,456,953 | 12/1948 | Knott et al    |
| 2,592,250   | 4/1952  | Davey et al    |
| 2,839,405   | 6/1958  | Jones          |
| 3,206,313   | 9/1965  | Porter et al   |
| 3,269,927   | 8/1966  | Atwell         |
| 3,448,709   | 6/1969  | Sidebotham     |
| 3,761,266   | 9/1973  | Milton         |
| 3,761,276   | 9/1973  | Evans          |
| 3,850,637   | 11/1974 | Evans          |
| 3,923,513   | 12/1975 | Evans          |
| 4,035,185   | 7/1977  | Atwell et al-- |

Signed and Sealed this  
*Eighteenth* Day of *March 1986*

[SEAL]

Attest:

DONALD J. QUIGG

Attesting Officer

Commissioner of Patents and Trademarks